



US009631160B2

(12) **United States Patent**  
**Burrington et al.**

(10) **Patent No.:** **US 9,631,160 B2**  
(45) **Date of Patent:** **\*Apr. 25, 2017**

(54) **STABILIZED BLENDS CONTAINING  
FRICTION MODIFIERS**

(75) Inventors: **James D. Burrington**, Gates Mills, OH (US); **Patrick E. Mosier**, Bay Village, OH (US); **David C. Arters**, Solon, OH (US); **Stuart L. Bartley**, Wickliffe, OH (US)

(73) Assignee: **The Lubrizol Corporation**, Wickliffe, OH (US)

(\*) Notice: Subject to any disclaimer, the term of this patent is extended or adjusted under 35 U.S.C. 154(b) by 0 days.

This patent is subject to a terminal disclaimer.

(21) Appl. No.: **14/114,761**

(22) PCT Filed: **May 22, 2012**

(86) PCT No.: **PCT/US2012/038921**

§ 371 (c)(1),  
(2), (4) Date: **Oct. 30, 2013**

(87) PCT Pub. No.: **WO2012/162282**

PCT Pub. Date: **Nov. 29, 2012**

(65) **Prior Publication Data**

US 2014/0080743 A1 Mar. 20, 2014

**Related U.S. Application Data**

(60) Provisional application No. 61/490,241, filed on May 26, 2011.

(51) **Int. Cl.**

**C07C 55/02** (2006.01)

**C10M 169/06** (2006.01)

**C10M 115/08** (2006.01)

**C10M 133/16** (2006.01)

**C10L 1/14** (2006.01)

**C10L 10/18** (2006.01)

**C10M 133/00** (2006.01)

**C10M 133/02** (2006.01)

**C10M 161/00** (2006.01)

**C10L 1/222** (2006.01)

**C10L 1/224** (2006.01)

**C10L 1/238** (2006.01)

**C10L 1/2387** (2006.01)

(52) **U.S. Cl.**

CPC ..... **C10M 133/16** (2013.01); **C10L 1/14**

(2013.01); **C10L 10/18** (2013.01); **C10M**

**133/00** (2013.01); **C10M 133/02** (2013.01);

**C10M 161/00** (2013.01); **C10L 1/224**

(2013.01); **C10L 1/2222** (2013.01); **C10L**

**1/2225** (2013.01); **C10L 1/2381** (2013.01);  
**C10L 1/2387** (2013.01); **C10M 2203/1006**  
(2013.01); **C10M 2207/124** (2013.01); **C10M**  
**2207/128** (2013.01); **C10M 2207/289**  
(2013.01); **C10M 2215/04** (2013.01); **C10M**  
**2215/042** (2013.01); **C10M 2215/08** (2013.01);  
**C10M 2215/082** (2013.01); **C10M 2215/086**  
(2013.01); **C10M 2215/26** (2013.01); **C10M**  
**2217/043** (2013.01); **C10N 2230/02** (2013.01);  
**C10N 2230/66** (2013.01)

(58) **Field of Classification Search**

CPC ..... C10M 2223/043; C10M 2207/028; C10M  
2219/046; C10M 2215/0813; C10M  
2215/02  
USPC ..... 508/506, 551, 521, 527  
See application file for complete search history.

(56) **References Cited**

**U.S. PATENT DOCUMENTS**

|                  |         |                                      |
|------------------|---------|--------------------------------------|
| 6,277,158 B1     | 8/2001  | McLean                               |
| 7,935,664 B2     | 5/2011  | Dowding et al.                       |
| 2003/0009930 A1  | 1/2003  | DeRosa et al.                        |
| 2005/0215441 A1* | 9/2005  | Mackney ..... C10M 133/08<br>508/291 |
| 2006/0079413 A1  | 4/2006  | Kocsis et al.                        |
| 2008/0026973 A1* | 1/2008  | Nelson et al. ..... 508/547          |
| 2008/0113890 A1* | 5/2008  | Moreton et al. ..... 508/547         |
| 2009/0270284 A1* | 10/2009 | Kikuchi et al. ..... 508/108         |
| 2010/0144565 A1  | 6/2010  | Ikeda et al.                         |
| 2010/0286007 A1  | 11/2010 | Kocsis et al.                        |

**FOREIGN PATENT DOCUMENTS**

|    |                  |        |         |
|----|------------------|--------|---------|
| WO | WO 2008147704 A1 | *      | 12/2008 |
| WO | 2010/005921 A1   | 1/2010 |         |
| WO | 2010/039509 A2   | 4/2010 |         |
| WO | 2011/066141 A1   | 6/2011 |         |
| WO | 2011/066142 A1   | 6/2011 |         |

\* cited by examiner

*Primary Examiner* — Vishal Vasisth

(74) *Attorney, Agent, or Firm* — Christopher D. Hilker;  
Teresan W. Gilbert

(57) **ABSTRACT**

The present invention relates to functional fluid compositions containing friction modifiers, and specifically stable compositions containing friction modifiers with limited solubility in and/or limited compatibility with the functional fluids with which they are used. In particular the present invention deals with functional fluids used in internal combustion engines, such as engine oils, and friction modifiers that contain one or more amide functional groups, where the friction modifier is present in the functional fluid composition at levels that would otherwise cause the composition to be unstable and/or hazy.

**16 Claims, No Drawings**

## 1

STABILIZED BLENDS CONTAINING  
FRICTION MODIFIERSCROSS REFERENCE TO RELATED  
APPLICATION

This application claims priority from PCT Application Serial No. PCT/US2012/038921 filed on May 22, 2012, which claims the benefit of U.S. Provisional Application No. 61/490,241 filed on May 26, 2011.

## BACKGROUND OF THE INVENTION

The present invention relates to functional fluid compositions containing friction modifiers, and specifically stable compositions containing friction modifiers with limited solubility in and/or limited compatibility with the functional fluids with which they are used.

Friction modifiers and their importance to various types of functional fluids are known. However, many friction modifiers may only be used in limited ways due to solubility and/or compatibility issues with the functional fluids in which they are used. Many friction modifiers, and specifically those containing amide groups, have limited solubility in functional fluids, such as engine oils and gear oils. These friction modifiers, when used at levels above their solubility and/or compatibility limits, may fall out of the functional fluid composition over time and/or cause the composition to appear hazy or cloudy.

These are serious issues in the manufacturing and blending processes of the fluids as well as in the field. For example, a functional fluid additive manufacturer would sell a homogeneous additive package of performance chemicals, which may then be added to a base oil to give a final lubricant, which in turn is sold in tanks, drums, cans and plastic containers for final delivery of the lubricant to the equipment to be lubricated. To maintain assurance of performance of the final lubricant, or any other functional fluid, in the equipment in which it is used, the concentrate and the lubricant must remain homogeneous throughout these steps. In other words, all of the additives present must be compatible with each of the various materials it comes into contact with and/or finds itself, from the additive package to the concentrate to the final fluid. This stringent standard greatly limits the choices of and available treatment levels for many additives, including the friction modifiers discussed herein. These friction modifiers could provide improved performance to a functional fluid but not widely used and/or are not used at the optimal level because the additive does not meet the solubility and/or compatibility requirements discussed above.

In the field, functional fluid compositions that drop out one or more components over time may not perform properly unless they are well-mixed before use, or may be removed by filters associated with the equipment in which the functional fluid is used. The haziness and/or cloudiness of a functional fluid, which may be measured as the fluid's turbidity, is often seen as a sign the composition is not stable, or may be in an early stage of separation and/or component drop out. Such conditions are not desired in functional fluid compositions, for both performance and aesthetic related reasons. This reality has created constraints on the use of various friction modifiers, such as effective maximum treat rates.

Without these solubility and/or compatibility limitations on the use of these friction modifiers, greater performance and equipment protection might be achievable, including for

## 2

example extended life of a lubricant or a lubricated piece of equipment such as engines, automatic transmissions, gear assemblies and the like. Improved fuel economy and viscosity stability might be achievable as well. Greater performance may even be achievable with lesser amounts of chemical as well as greater amounts, depending on the selection of the more effective, but otherwise not suitable chemicals from a compatibility or solubility standpoint when delivered in a conventional manner.

10 There is a need for functional fluid compositions that contain higher amounts of friction modifiers while still remaining stable and/or clear. There is particularly a need for functional fluid compositions, such as engine oil compositions, that contain friction modifiers containing amide groups, at levels that would otherwise cause the composition to be unstable and/or hazy, as described above. The compositions and methods of the present invention overcome these constraints and thus allow the use of these friction modifiers at levels not otherwise possible while still maintaining the stability and/or clarity of the functional fluid composition.

## SUMMARY OF THE INVENTION

25 Functional fluid compositions have been discovered that may contain high amounts of friction modifiers, and particularly friction modifiers with limited solubility in and/or compatibility with the functional fluid compositions in which they are used, allowing for the use of higher amounts 30 of such friction modifiers in these functional fluid compositions, while maintaining the stability, clarity, and/or compatibility of the overall composition.

35 The present invention provides a composition that includes: (a) a medium, which may include a solvent, a functional fluid, or combinations thereof; and (b) a friction modifier component that includes a compound containing one or more amide functional groups that is not fully soluble in the medium; and (c) a stabilizing component that is soluble in (a) and that interacts with (b) such that (b)'s 40 solubility in (a) is improved, or perhaps more accurately, (b)'s solubility in the combination of (a) and (b) is improved over (b)'s solubility in the combination of (a) and (b) is improved over (b)'s solubility in (a) where the stabilizing component includes a compound having at least one hydrogen-donating group, a least one hydrogen-accepting group, and at least one hydrocarbyl group, where the hydrogen-donating group and the hydrogen-accepting group are not separated by more than 8 covalent and ionic bonds. Components (b) and (c) may be present in component (a) in the 45 form of dispersed particles having an average diameter of less than 10 microns.

50 The invention provides for the compositions described herein where the turbidity of the overall composition is improved, as defined by visual clarity ratings (such as shown in Tables 1-3 below), or a lower JTU and/or NTU value 55 compared to the same composition that does not contain (c), the stabilizing component. In some embodiments the compositions of the present invention have a maximum JTU and/or NTU value of 100.

60 The present invention also provides for a process of preparing a clear and stable composition, as described herein, said method including the steps of: (I) adding components (b) and (c) to component (a); and (II) mixing the components so that particles of components (b) and (c), or 65 in some embodiments particles of component (b) alone, have an average diameter of less than 10 microns, or in other embodiments and more specifically, no more than 10 percent

by weight of the particles have a diameter of more than 0.5 microns. In addition, component (b) may be present in the overall composition at a minimum amount, such as no less than 0.15 percent by weight.

The invention also provides the use of the compatibilizers and compositions described herein to improve the solubility and/or compatibility and/or stability of compositions containing the friction modifiers described herein.

#### DETAILED DESCRIPTION OF THE INVENTION

Various preferred features and embodiments will be described below by way of non-limiting illustration.

The present invention provides compositions, methods and uses that allow for the use of certain friction modifiers in functional fluid compositions that could not otherwise be used, and/or could not be used at the levels allowed for by the present invention, without resulting in unstable, unclear, and/or hazy compositions.

The types of functional fluids in and with which the compositions and methods of the present invention may be used can include: gear oils, transmission oils, hydraulic fluids, engine oils, two cycle oils, metalworking fluid, fuels and the like. In one embodiment the functional fluid is engine oil. In another embodiment the functional fluid is gear oil. In another embodiment the functional fluid is a transmission fluid. In another embodiment the functional fluid is a hydraulic fluid. In another embodiment the functional fluid is a fuel.

In some embodiments the present invention does not include the use of a delivery device, for example a device that acts to contain the friction modifier and contact it with the functional fluid with which it is to be added. In some embodiments the present invention does not include the use of either a gel composition or a solid composition, where such compositions slow release one or more components into a functional fluid. Rather the present invention provides a means for incorporating friction modifiers into functional fluids, by use of a combination of components, which result in a functional fluid with the high level of friction modifier while still being stable, clear and/or non-hazy.

In some embodiments the present invention provides a composition that is more stable, clearer, and/or less hazy than a composition that is identical except for it missing one or more components. In some embodiments the missing component is the stabilizing component. In other embodiments the compositions of the present invention have a lower turbidity compared to compositions that are identical except for them missing the stabilizing component of the present invention. In some of these embodiments, the compositions' turbidity is expressed as a visual clarity rating such as in Tables 1-3 or a JTU and/or NTU value. In other embodiments the compositions of the present invention have a maximum JTU and/or NTU value of 100, of 90 or even of 80.

JTU and NTU values may be measured US EPA method 180.1. JTU and NTU values may also be measured without any further dilution in Jackson Turbidity Units (JTU's) by using a Monitek Model 151 Turbidimeter.

#### The Medium

The compositions of the present invention include a medium. The medium may be a solvent, a functional fluid, an additive concentrate, or combinations thereof.

Suitable solvents include aliphatic hydrocarbons, aromatic hydrocarbons, oxygen containing compositions, or mixtures thereof. The oxygen containing composition can

include an alcohol, a ketone, an ester of a carboxylic acid, a glycol and/or a polyglycol, or a mixture thereof. Suitable solvents also include oils of lubricating viscosity, naphtha, toluene, xylene, or combinations thereof. The oil of lubricating viscosity can comprise natural oils, synthetic oils, or mixtures thereof. The oil of lubricating viscosity can be an API (American Petroleum Institute) Group II, III, IV, V base oil or mixture thereof. Examples of commercially available aliphatic hydrocarbon solvents or diluents, to include oils of lubricating viscosity, are Pilot™ 140 and Pilot™ 299 and Pilot™ 900 available from Petrochem Carless, Petro-Canadat™ 100N, Nexbase™, Yubase™, and 4 to 6 cSt poly(alpha-olefins).

Suitable functional fluids include any of the functional fluids listed above, including mixtures of such fluids. In many embodiments the functional fluids, or other materials used as the medium, contain additional additives in addition to components (b) and (c) described in detail below. These additional additives are described in greater detail below.

In one embodiment of the invention the medium and/or the overall composition is substantially free of or free of at least one member selected from the group consisting of sulphur, phosphorus, sulfated ash, and combinations thereof, and in other embodiments the fuel composition contains less than 20 ppm, less than 15 ppm, less than 10 ppm, or less than 1 ppm of at least one member selected from the group consisting of sulphur, phosphorus, sulfated ash, and combinations thereof.

In one embodiment, the medium and the stabilizing component may be similar materials. That is a material of the same type may perform the functions of both components. For example when the invention is in the form of a concentrate the medium present may act as a stabilizing component and vice versa. This concentrate may then be added to a functional fluid as a top treat and/or additive package, resulting in a stable and homogeneous functional fluid which would otherwise be cloudy or incompatible in the absence of stabilizer component/medium material.

#### The Friction Modifier

The compositions of the present invention include a friction modifier component. The friction modifier component may include at least one friction modifier that is not fully soluble and/or compatible in the medium and/or functional fluid in which it is to be used. By not fully soluble and/or compatible, it is meant that the friction modifier does not stay dissolved and/or suspended in the fluid to which it is added, causes the fluid to appear hazy and/or cloudy, have sediments, or any combination thereof. In some embodiments, the friction modifier causes the fluid in which it is used to have hazy appearance or solid drop-out, or an NTU and/or JTU value above 80, 90 or even 100. In some embodiments this fluid is a functional fluid composition such as a finished lubricant or an additive concentrate.

In some embodiments the friction modifier of the present invention is soluble and/or compatible with a fluid at low concentrations, but becomes less than soluble and/or compatible at higher concentrations. In some embodiments friction modifiers suitable for use in the present invention are not fully soluble and/or compatible, as defined above, when present in a fluid at concentrations of or more than 0.1, 0.15, 0.2, 0.3, 0.5, or 1.0 percent by weight.

In some embodiments the friction modifier of the present invention comprises a compound containing one or more amide functional groups. Suitable friction modifiers include compounds represented by the formula:



wherein: X⁴ is an oxygen atom or a sulfur atom; and each R² and R³ is independently a hydrogen or a hydrocarbyl group. Examples of suitable friction modifiers include oleyl amide, stearyl amide, or combinations thereof.

Fatty acid amides have been discussed in detail in U.S. Pat. No. 4,280,916. Suitable amides are C<sub>8</sub>-C<sub>24</sub> aliphatic monocarboxylic amides and are well known. Reacting the fatty acid based compound with ammonia or an amine produces the fatty amide. The fatty acids and amides derived there from may be either saturated or unsaturated. Important fatty acids include lauric acid (C<sub>12</sub>), palmitic acid (C<sub>16</sub>), and steric acid (C<sub>18</sub>). Other important unsaturated fatty acids include oleic, linoleic and linolenic acids, all of which are C<sub>18</sub>. In one embodiment, the fatty amides of the instant invention are those derived from the C<sub>18</sub> unsaturated fatty acids.

The fatty amines and the diethoxylated long chain amines such as N,N-bis-(2-hydroxyethyl)-tallowamine themselves are generally useful as friction modifier components of this invention. Both types of amines are commercially available. Fatty amines and ethoxylated fatty amines are described in greater detail in U.S. Pat. No. 4,741,848.

The friction modifier may be present in the compositions of the present invention at levels of at least 0.05, 0.1, 0.15, 0.2, 0.3, 0.5 or even 1.0 percent by weight. The friction modifier may be present at amounts up to, or even less than, 10, 9, 8, 7.5, 5, or even 4 or 3 percent by weight.

The compositions of the present invention, and specifically the friction modifier component, may optionally include one or more additional friction modifiers. These additional friction modifiers may or may not have the solubility and/or compatibility issues of the friction modifiers described above. These additional friction modifiers may include esters of polyols such as glycerol monooleate, as well as there borated derivatives; fatty phosphites; borated fatty epoxides; sulfurized olefins; compounds derived from a hydroxy-carboxylic acid such as oleyl tartramide, stearyl tartramide, and 2-ethylhexyl tartrate; and mixtures thereof.

Esters of polyols include fatty acid esters of glycerol. These can be prepared by a variety of methods well known in the art. Many of these esters, such as glycerol monooleate and glycerol mono-tallowate, are manufactured on a commercial scale. The esters useful for this invention are oil-soluble and are preferably prepared from C<sub>8</sub> to C<sub>22</sub> fatty acids or mixtures thereof such as are found in natural products. The fatty acid may be saturated or unsaturated. Certain compounds found in acids from natural sources may include licanic acid which contains one keto group. Useful C<sub>8</sub> to C<sub>22</sub> fatty acids are those of the formula R—COOH wherein R is alkyl or alkenyl.

The fatty acid monoester of glycerol is useful. Mixtures of mono and diesters may be used. Mixtures of mono- and diester can contain at least about 40% of the monoester. Mixtures of mono- and diesters of glycerol containing from about 40% to about 60% by weight of the monoester can be used. For example, commercial glycerol monooleate containing a mixture of from 45% to 55% by weight monoester and from 55% to 45% diester can be used.

Useful fatty acids for making these fatty acid esters include oleic, stearic, isostearic, palmitic, myristic, palmitoleic, linoleic, lauric, linolenic, and eleostearic, and the acids from the natural products tallow, palm oil, olive oil, peanut oil.

Friction modifiers derived from a hydroxy-carboxylic acid may be formed by the reaction of the acid with an alcohol and/or an amine. Suitable hydroxy-carboxylic acid include those represented by the formula:



wherein: a and b may be independently integers of 1 to 5, or 1 to 2; X may be an aliphatic or alicyclic group, or an aliphatic or alicyclic group containing an oxygen atom in the carbon chain, or a substituted group of the foregoing types, said group containing up to 6 carbon atoms and having a+b available points of attachment; each Y may be independently —O—, >NH, or >NR³ or two Y's together representing the nitrogen of an imide structure R¹—N< formed between two carbonyl groups; and each R¹ and R³ may be independently hydrogen or a hydrocarbyl group, provided that at least one R¹ and R³ group may be a hydrocarbyl group; each R² may be independently hydrogen, a hydrocarbyl group or an acyl group, further provided that at least one —OR² group is located on a carbon atom within X that is α or β to at least one of the —C(O)—Y—R¹ groups.

In one embodiment the acid is represented by the formula:



wherein each R⁴ is independently H or a hydrocarbyl group, or wherein the R⁴ groups together form a ring. In one embodiment the friction modifier is borated. In another embodiment the friction modifier is not borated.

In any of the embodiments above, the hydroxy-carboxylic acid may be tartaric acid, citric acid, or combinations thereof, and may also be a reactive equivalent of such acids (including esters, acid halides, or anhydrides). The resulting friction modifiers may include imide, di-ester, di-amide, or ester-amide derivatives of tartaric acid, citric acid, or mixtures thereof. In one embodiment the derivative of hydroxy-carboxylic acid includes an imide, a di-ester, a di-amide, or an ester-amide derivative of tartaric acid.

The amines used in the preparation of the friction modifier may have the formula RR'NH wherein R and R' each independently represent H, a hydrocarbon-based radical of 1 or 8 to 30 or 150 carbon atoms, that is, 1 to 150 or 8 to 30 or 1 to 30 or 8 to 150 atoms. Amines having a range of carbon atoms with a lower limit of 2, 3, 4, 6, 10, or 12 carbon atoms and an upper limit of 120, 80, 48, 24, 20, 18, or 16 carbon atoms may also be used. In one embodiment, each of the groups R and R' has 8 or 6 to 30 or 12 carbon atoms. In one embodiment, the sum of carbon atoms in R and R' is at

least 8. R and R' may be linear or branched. In one embodiment R and R' are linear and have at least 12 carbons. In such embodiments the groups may include some unsaturation.

The alcohols useful for preparing the friction modifier will similarly contain 1 or 8 to 30 or 150 carbon atoms. Alcohols having a range of carbon atoms from a lower limit of 2, 3, 4, 6, 10, or 12 carbon atoms and an upper limit of 120, 80, 48, 24, 20, 18, or 16 carbon atoms may also be used. In certain embodiments the number of carbon atoms in the alcohol-derived group may be 8 to 24, 10 to 18, 12 to 16, or 13 carbon atoms.

The alcohols and amines may be linear or branched, and, if branched, the branching may occur at any point in the chain and the branching may be of any length. In some embodiments the alcohols and/or amines used include branched compounds, and in still other embodiments, the alcohols and amines used are at least 50%, 75% or even 80% branched.

In some embodiments, the alcohol and/or amine used includes branched C<sub>6-18</sub> or C<sub>8-18</sub> alcohols, branched C<sub>12-16</sub> alcohols, 2-ethylhexanol, isotridecyl alcohol, linear C<sub>6-18</sub> or C<sub>8-18</sub> alcohols, linear C<sub>12-16</sub> alcohols, or combinations thereof.

In one embodiment the hydroxy-acid derived friction modifier can be represented by a compound of the formula:



wherein: n' is 0 to 10; p is 1 to 5; Y and Y' are independently —O—, >NH, >NR<sup>7</sup>, or an imide group formed by the linking of the Y and Y' groups forming a R<sup>1</sup>—N< group between two >C=O groups; R<sup>5</sup> and R<sup>6</sup> are independently hydrocarbyl groups, typically containing 1, 4 or 6 to 150, 30 or 24 carbon atoms; m is 0 or 1, and X is independently —CH<sub>2</sub>—, >CHR<sup>8</sup> or >CR<sup>8</sup>R<sup>9</sup>, >CHOR<sup>10</sup>, or >C(CO<sub>2</sub>R<sup>10</sup>)<sub>2</sub>, —CH<sub>3</sub>, —CH<sub>2</sub>R<sup>8</sup> or —CHR<sup>8</sup>R<sup>9</sup>, —CH<sub>2</sub>OR<sup>10</sup>, or —CH(CO<sub>2</sub>R<sup>10</sup>)<sub>2</sub>, or mixtures thereof wherein: R<sup>7</sup> is a hydrocarbyl group; R<sup>8</sup> and R<sup>9</sup> are independently keto-containing groups (such as acyl groups), ester groups or hydrocarbyl groups; and R<sup>10</sup> is independently hydrogen or a hydrocarbyl group, typically containing 1 to 150 carbon atoms.

In some embodiments the compounds represent by Formula IV have at least one X that is hydroxyl-containing (e.g., >CHOR<sup>10</sup>, wherein R<sup>10</sup> is hydrogen). When X is hydroxyl-containing, the compound may be derived from hydroxy-carboxylic acids such as tartaric acid, citric acid, or mixtures thereof. In one embodiment the compound is derived from citric acid and R<sup>5</sup> and R<sup>6</sup> contain at least 6 or 8 carbon atoms up to 150, or 6 or 8 to 30 or 24 carbon atoms. In one embodiment the compound is derived from tartaric acid and R<sup>5</sup> and R<sup>6</sup> contain 4 or 6 to 30 or 24 carbon atoms. When X is not hydroxyl-containing, the compound may be derived from malonic acid, oxalic acid, chlorophenyl malonic acid, reactive equivalents thereof such as esters, or mixtures thereof.

In some embodiments the compositions of the present invention do not include any of these optional friction modifiers and in other embodiments, one or more of any of the optional friction modifiers listed herein are not present in the compositions of the present invention.

In other embodiments an additional friction modifier is present, and that friction modifier is derived from a hydroxy-

acid. In other embodiments the additional friction modifier is oleyl tartrimide, stearyl tartrimide, 2-ethylhexyl tartrimide, or combinations thereof.

The additional friction modifier may be present in the compositions of the present invention at levels of at least 0.05, 0.1, 0.15, 0.2, 0.3, 0.5 or even 1.0 percent by weight. The additional friction modifier may be present at less than 10, 7.5, 5, or even 4 or 3 percent by weight.

#### The Stabilizing Component

10 The compositions of the present invention include a stabilizing component. The stabilizing component of the present invention is soluble in medium and that interacts with the friction modifier such that its solubility in the medium and/or overall composition is improved. This may be accomplished by an association of the stabilizing component and the friction modifier, resulting in suspended particles of the associated molecules, that remain suspended, dispersed and/or dissolved in the medium and/or overall composition to an extent greater than obtained by the friction modifier alone.

15 The stabilizing component of the present invention is an additive that, when combined with the friction modifier in the medium, results in an improvement in the turbidity of the composition, compared to the same composition that does not contain the stabilizing component. The stabilizing component comprises a compound having at least one hydrogen-donating group, a least one hydrogen-accepting group, and at least one hydrocarbyl group, where the hydrogen-donating group and the hydrogen-accepting group are not separated by more than 8 covalent and ionic bonds.

20 In some embodiments the stabilizing component includes a quaternary salt comprising the reaction product of (a) hydrocarbyl-substituted compound having a tertiary amino group and (b) a quaternizing agent suitable for converting the tertiary amino group of (a) to a quaternary nitrogen, wherein the quaternizing agent is selected from the group consisting of dialkyl sulfates, benzyl halides, hydrocarbyl substituted carbonates; hydrocarbyl epoxides in combination with an acid or mixtures thereof.

25 30 35 40 The quaternary salt may include the reaction product of: (i) at least one compound selected from the group consisting of: (a) the condensation product of a hydrocarbyl-substituted acylating agent and a compound having an oxygen or nitrogen atom capable of condensing with said acylating agent and said condensation product further having a tertiary amino group; (b) a polyalkene-substituted amine having at least one tertiary amino group; and (c) a Mannich reaction product having a tertiary amino group, said Mannich reaction product being prepared from the reaction of a hydrocarbyl-substituted phenol, an aldehyde, and an amine; and (ii) a quaternizing agent suitable for converting the tertiary amino group of compound (i) to a quaternary nitrogen, wherein the quaternizing agent is selected from the group consisting of dialkyl sulfates, benzyl halides, hydrocarbyl substituted carbonates; hydrocarbyl epoxides in combination with an acid or mixtures thereof.

45 50 55 In one embodiment the quaternary salt comprises the reaction product of (i) at least one compound selected from the group consisting of: a polyalkene-substituted amine having at least one tertiary amino group and/or a Mannich reaction product having a tertiary amino group; and (ii) a quaternizing agent.

60 65 In another embodiment the quaternary salt comprises the reaction product of (i) the reaction product of a succinic anhydride and an amine; and (ii) a quaternizing agent. In such embodiments, the succinic anhydride may be derived from polyisobutylene and an anhydride, where the poly-

isobutylene has a number average molecular weight of about 800 to about 1600. In some embodiments the succinic anhydride is chlorine free.

In some embodiments, the hydrocarbyl substituted acylating agent of component (i)(a) described above is the reaction product of a long chain hydrocarbon, generally a polyolefin substituted with a monounsaturated carboxylic acid reactant such as (1) monounsaturated C<sub>4</sub> to C<sub>10</sub> dicarboxylic acid such as fumaric acid, itaconic acid, maleic acid; (2) derivatives of (1) such as anhydrides or C<sub>1</sub> to C<sub>5</sub> alcohol derived mono- or di-esters of (1); (3) monounsaturated C<sub>3</sub> to C<sub>10</sub> monocarboxylic acid such as acrylic acid and methacrylic acid; or (iv) derivatives of (3) such as C<sub>1</sub> to C<sub>5</sub> alcohol derived esters of (3) with any compound containing an olefinic bond represented by the general formula:



wherein each R<sup>1</sup> is independently hydrogen or a hydrocarbyl group.

Olefin polymers for reaction with the monounsaturated carboxylic acids can include polymers comprising a major molar amount of C<sub>2</sub> to C<sub>20</sub>, e.g. C<sub>2</sub> to C<sub>5</sub> monoolefin. Such olefins include ethylene, propylene, butylene, isobutylene, pentene, octene-1, or styrene. The polymers can be homopolymers such as polyisobutylene, as well as copolymers of two or more of such olefins such as copolymers of; ethylene and propylene; butylene and isobutylene; propylene and isobutylene. Other copolymers include those in which a minor molar amount of the copolymer monomers e.g., 1 to 10 mole % is a C<sub>4</sub> to C<sub>18</sub> diolefin, e.g., a copolymer of isobutylene and butadiene; or a copolymer of ethylene, propylene and 1,4-hexadiene.

In one embodiment, at least one R of formula of the compound containing an olefinic bond provided above is derived from polybutene, that is, polymers of C<sub>4</sub> olefins, including 1-butene, 2-butene and isobutylene. C<sub>4</sub> polymers can include polyisobutylene. In another embodiment, at least one R of compound containing an olefinic bond is derived from ethylene-alpha olefin polymers, including ethylene-propylene-diene polymers. Ethylene-alpha olefin copolymers and ethylene-lower olefin-diene terpolymers are described in numerous patent documents, including European patent publication EP0279863 and the following U.S. Pat. Nos.: 3,598,738; 4,026,809; 4,032,700; 4,137,185; 4,156,061; 4,320,019; 4,357,250; 4,658,078; 4,668,834; 4,937,299; 5,324,800 each of which are incorporated herein by reference for relevant disclosures of these ethylene based polymers.

In another embodiment, the olefinic bonds of the compound containing an olefinic bonds described above are predominantly vinylidene groups, represented by the following formulas:



wherein R<sup>2</sup> is a hydrocarbyl group, and in some embodiments both R<sup>2</sup> groups are methyl groups, and



wherein R<sup>3</sup> is a hydrocarbyl group.

In one embodiment, the vinylidene content of the formula of the compound containing an olefinic bond provided above can comprise at least about 30 mole % vinylidene groups, at least about 50 mole % vinylidene groups, or at least about 70 mole % vinylidene groups. Such material and methods for preparing them are described in U.S. Pat. Nos. 5,071,919; 5,137,978; 5,137,980; 5,286,823, 5,408,018, 6,562,913, 6,683,138, 7,037,999 and U.S. Publication Nos.

20040176552A1, 20050137363 and 20060079652A1, which are expressly incorporated herein by reference, such products are commercially available by BASF, under the trademark GLISSOPAL® and by Texas Petrochemicals LP, under the trademark TPC 1105™ and TPC 595™.

Methods of making hydrocarbyl substituted acylating agents from the reaction of the monounsaturated carboxylic acid reactant and the compound containing an olefinic bond described above are well known in the art and disclosed in the following patents: U.S. Pat. Nos. 3,361,673 and 3,401,118 to cause a thermal "ene" reaction to take place; U.S. Pat. Nos. 3,087,436; 3,172,892; 3,272,746, 3,215,707; 3,231,587; 3,912,764; 4,110,349; 4,234,435; 6,077,909; 6,165,235 and are hereby incorporated by reference.

In another embodiment, the hydrocarbyl substituted acylating agent can be made from the reaction of at least one carboxylic reactant represented by the following formulas:



and



wherein each R<sup>4</sup> is independently H or a hydrocarbyl group, and each R<sup>5</sup> is a divalent hydrocarbylene group and n is 0 or 1 with any compound containing an olefin bond as described above. Compounds and the processes for making these compounds are disclosed in U.S. Pat. Nos. 5,739,356; 5,777,142; 5,786,490; 5,856,524; 6,020,500; and 6,114,547 which are hereby incorporated by reference.

Other methods of making the hydrocarbyl substituted acylating agent can be found in the following reference, U.S. Pat. Nos. 5,912,213; 5,851,966; and 5,885,944 which are hereby incorporated by reference.

The compound having an oxygen or nitrogen atom capable of condensing with the acylating agent and further having a tertiary amino group can be represented by the following formulas:



wherein X is an alkylene group containing about 1 to about 4 carbon atoms; and wherein each R<sup>6</sup> is independently a hydrocarbyl group, and R<sup>6</sup> can be hydrogen or a hydrocarbyl group.



wherein X is an alkylene group containing about 1 to about 4 carbon atoms; and wherein each R<sup>7</sup> is independently a hydrocarbyl group.

Examples of the nitrogen or oxygen contain compounds capable of condensing with the acylating agent and further

11

having a tertiary amino group can include but are not limited to: ethylenediamine, 1,2-propylenediamine, 1,3-propylene diamine, the isomeric butylenediamines, pentanediamines, hexanediamines, heptanediamines, diethylenetriamine, dipropylenetriamine, dibutylenetriamine, triethylenetriamine, tetraethylenepentaamine, pentaethylenehexaamine, hexamethylenetetramine, and bis(hexamethylene) triamine, the diaminobenzenes, the diaminopyridines or mixtures thereof. In addition, nitrogen or oxygen contain compounds which may be alkylated to contain a tertiary amino group may also used. Examples of the nitrogen or oxygen contain compounds capable of condensing with the acylating agent after being alkylated to having a tertiary amino group can include but are not limited to: dimethylaminopropylamine, N,N-dimethyl-aminopropylamine, N,N-diethyl-aminopropylamine, N,N-dimethyl-aminoethylamine or mixtures thereof. The nitrogen or oxygen containing compounds capable of condensing with the acylating agent and further having a tertiary amino group can further include aminoalkyl substituted heterocyclic compounds such as 1-(3-aminopropyl)imidazole and 4-(3-aminopropyl)morpholine, 1-(2-aminoethyl)piperidine, 3,3-diamino-N-methylpropylamine, 3'3-aminobis(N,N-dimethylpropylamine). Another type of nitrogen or oxygen containing compounds capable of condensing with the acylating agent and having a tertiary amino group include alkanolamines including but not limited to triethanolamine, N,N-dimethylaminopropanol, N,N-diethylaminopropanol, N,N-diethylaminobutanol, N,N,N-tris(hydroxethyl)amine, or mixtures thereof.

The acid used with the quaternizing agent may be an organic acid represented by the general formula  $R-COOH$  where  $R$  is a hydrocarbyl group. In some embodiments the hydrocarbyl group of the acid contains from 1 to 10, 1 to 6 or even 1 to 4 carbons atoms. In some embodiments the acid may be acetic acid, propionic acid, butyric acid, or pentanoic acid.

Examples of quaternary ammonium salt and methods for preparing the same are described in the following patents, which are hereby incorporated by reference, U.S. Pat. Nos. 4,253,980, 3,778,371, 4,171,959, 4,326,973, 4,338,206, and 5,254,138.

The quaternary salts of the invention may also comprise a polyester quaternary ammonium salt which may be derived from the reaction of a polyester that contains a tertiary amino group and a quaternizing agent suitable for converting the tertiary amino group to a quaternary nitrogen.

The polyester containing a tertiary amino group used in the preparation of the additives of the invention may also be described as a non-quaternized polyester containing a tertiary amino group.

In some embodiments the polyester is the reaction product of a fatty carboxylic acid containing at least one hydroxyl group and a compound having an oxygen or nitrogen atom capable of condensing with said acid and further having a tertiary amino group. Suitable fatty carboxylic acids that may be used in the preparation of the polyesters described above may be represented by the formula:



where  $R^1$  is a hydrogen or a hydrocarbyl group containing from 1 to 20 carbon atoms and  $R^2$  is a hydrocarbylene group containing from 1 to 20 carbon atoms. In some embodiments

12

$R^1$  contains from 1 to 12, 2 to 10, 4 to 8 or even 6 carbon atoms, and  $R^2$  contains from 2 to 16, 6 to 14, 8 to 12, or even 10 carbon atoms.

In some embodiments the fatty carboxylic acid used in the preparation of the polyester is 12-hydroxystearic acid, ricinoleic acid, 12-hydroxy dodecanoic acid, 5-hydroxy dodecanoic acid, 5-hydroxy decanoic acid, 4-hydroxy decanoic acid, 10-hydroxy undecanoic acid, or combinations thereof.

The compound having an oxygen or nitrogen atom capable of condensing with said acid and further having a tertiary amino group may include any of the materials described above as compounds having an oxygen or nitrogen atom capable of condensing with the acylating agent. Suitable materials may be represented by the formula:



where  $R^3$  is a hydrocarbyl group containing from 1 to 10 carbon atoms;  $R^4$  is a hydrocarbyl group containing from 1 to 10 carbon atoms;  $R^5$  is a hydrocarbylene group containing from 1 to 20 carbon atoms; and  $X^1$  is O or  $NR^6$  where  $R^6$  is a hydrogen or a hydrocarbyl group containing from 1 to 10 carbon atoms. In some embodiments  $R^3$  contains from 1 to 6, 1 to 2, or even 1 carbon atom,  $R^4$  contains from 1 to 6, 1 to 2, or even 1 carbon atom,  $R^5$  contains from 2 to 12, 2 to 8 or even 3 carbon atoms, and  $R^6$  contains from 1 to 8, or 1 to 4 carbon atoms. In some of these embodiments the compound becomes becomes:



where the various definitions provided above still apply.

Examples of nitrogen or oxygen containing compounds capable of condensing with the polyester agents include all of those listed above as examples of materials that are capable of condensing with the acylating agents.

The quaternized polyester salt can be a quaternized poly-ester amide salt. In such embodiments the polyester containing a tertiary amino group used to prepare the quaternized polyester salt is a polyester amide containing a tertiary amino group. In some of these embodiments the amine or amino alcohol is reacted with a monomer and then the resulting material is polymerized with additional monomer, resulting in the desired polyester amide which may then be quaternized.

In some embodiments the quaternized polyester salt includes an anion represented by the following formula:



where  $R^1$  is a hydrogen or a hydrocarbyl group containing from 1 to 20 carbon atoms and  $R^2$  is a hydrocarbylene group containing from 1 to 20 carbon atoms;  $R^3$  is a hydrocarbyl group containing from 1 to 10 carbon atoms;  $R^4$  is a

hydrocarbyl group containing from 1 to 10 carbon atoms; R<sup>5</sup> is a hydrocarbylene group containing from 1 to 20 carbon atoms; R<sup>6</sup> is a hydrogen or a hydrocarbyl group containing from 1 to 10 carbon atoms; n is a number from 1 to 10; R<sup>7</sup> is hydrogen, a hydrocarbyl group containing from 1 to 22 carbon atoms, or a hydrocarbyl group containing from 1 to 22 carbon atoms; and X<sup>2</sup> is a group derived from the quaternizing agent. In some embodiments R<sup>6</sup> is hydrogen.

As above, in some embodiments R<sup>1</sup> contains from 1 to 12, 2 to 10, 4 to 8 or even 6 carbon atoms, and R<sup>2</sup> contains from 2 to 16, 6 to 14, 8 to 12, or even 10 carbon atoms, R<sup>3</sup> contains from 1 to 6, 1 to 2, or even 1 carbon atom, R<sup>4</sup> contains from 1 to 6, 1 to 2, or even 1 carbon atom, R<sup>5</sup> contains from 2 to 12, 2 to 8 or even 3 carbon atoms, and R<sup>6</sup> contains from 1 to 8, or 1 to 4 carbon atoms. In any of these embodiments n may be from 2 to 9, or 3 to 7, and R<sup>7</sup> may contain from 6 to 22, or 8 to 20 carbon atoms.

In these embodiments the quaternized polyester salt is essentially capped with a C1-22, or a C8-20, fatty acid. Examples of suitable acids include oleic acid, palmitic acid, stearic acid, erucic acid, lauric acid, 2-ethylhexanoic acid, 9,11-linoleic acid, 9,12-linoleic acid, 9,12,15-linolenic acid, abietic acid, or combinations thereof.

The number average molecular weight (Mn) of the quaternized polyester salts of the invention may be from 500 to 3000, or from 700 to 2500.

The polyester useful in the present invention can be obtained by heating one or more hydroxycarboxylic acids or a mixture of the hydroxycarboxylic acid and a carboxylic acid, optionally in the presence of an esterification catalyst. The hydroxycarboxylic acids can have the formula HO—X—COOH wherein X is a divalent saturated or unsaturated aliphatic radical containing at least 8 carbon atoms and in which there are at least 4 carbon atoms between the hydroxy and carboxylic acid groups, or from a mixture of such a hydroxycarboxylic acid and a carboxylic acid which is free from hydroxy groups. This reaction can be carried out at a temperature in the region of 160 C. to 200 C., until the desired molecular weight has been obtained. The course of the esterification can be followed by measuring the acid value of the product, with the desired polyester, in some embodiments, having an acid value in the range of 10 to 100 mg KOH/g or in the range of 20 to 50 mg KOH/g. The indicated acid value range of 10 to 100 mg KOH/g is equivalent to a number average molecular weight range of 5600 to 560. The water formed in the esterification reaction can be removed from the reaction medium, and this can be conveniently done by passing a stream of nitrogen over the reaction mixture or, by carrying out the reaction in the presence of a solvent, such as toluene or xylene, and distilling off the water as it is formed.

The resulting polyester can then be isolated in conventional manner; however, when the reaction is carried out in the presence of an organic solvent whose presence would not be harmful in the subsequent application, the resulting solution of the polyester can be used.

In the said hydroxycarboxylic acids the radical represented by X may contain from 12 to 20 carbon atoms, optionally where there are between 8 and 14 carbon atoms between the carboxylic acid and hydroxy groups. In some embodiments the hydroxy group is a secondary hydroxy group.

Specific examples of such hydroxycarboxylic acids include ricinoleic acid, a mixture of 9- and 10-hydroxystearic acids (obtained by sulphation of oleic acid followed by hydrolysis), and 12-hydroxystearic acid, and especially the commercially available hydrogenated castor oil fatty

acid which contains in addition to 12-hydroxystearic acid minor amounts of stearic acid and palmitic acid.

The carboxylic acids which can be used in conjunction with the hydroxycarboxylic acids to obtain these polyesters are preferably carboxylic acids of saturated or unsaturated aliphatic compounds, particularly alkyl and alkenyl carboxylic acids containing a chain of from 8 to 20 carbon atoms. As examples of such acids there may be mentioned lauric acid, palmitic acid, stearic acid and oleic acid.

In one embodiment the polyester is derived from commercial 12-hydroxy-stearic acid having a number average molecular weight of about 1600. Polyesters such as this are described in greater detail in U.K. Patent Specification Nos. 1373660 and 1342746.

In some embodiments the components used to prepare the additives described above are substantially free of, essentially free of, or even completely free of, non-polyester-containing hydrocarbyl substituted acylating agents and/or non-polyester-containing hydrocarbyl substituted diacylating agents, such as for example polyisobutylene. In some embodiments these excluded agents are the reaction product of a long chain hydrocarbon, generally a polyolefin reacted with a monounsaturated carboxylic acid reactant, such as, (i) α,β-monounsaturated C<sub>4</sub> to C<sub>10</sub> dicarboxylic acid, such as, fumaric acid, itaconic acid, maleic acid; (ii) derivatives of (i) such as anhydrides or C<sub>1</sub> to C<sub>5</sub> alcohol derived mono- or di-esters of (i); (iii) α,β-monounsaturated C<sub>3</sub> to C<sub>10</sub> mono-carboxylic acid such as acrylic acid and methacrylic acid; or (iv) derivatives of (iii), such as, C<sub>1</sub> to C<sub>5</sub> alcohol derived esters of (iii) with any compound containing an olefinic bond represented by the general formula (R<sup>9</sup>)(R<sup>10</sup>)C=C(R<sup>11</sup>)CH(R<sup>7</sup>)(R<sup>8</sup>)) wherein each of R<sup>9</sup> and R<sup>10</sup> is independently hydrogen or a hydrocarbon based group; each of R<sup>11</sup>, R<sup>7</sup> and R<sup>8</sup> is independently hydrogen or a hydrocarbon based group and preferably at least one is a hydrocarbyl group containing at least 20 carbon atoms. In one embodiment, the excluded hydrocarbyl-substituted acylating agent is a dicarboxylic acylating agent. In some of these embodiments, the excluded hydrocarbyl-substituted acylating agent is polyisobutylene succinic anhydride.

By substantially free of, it is meant that the components of the present invention are primarily composed of materials other than hydrocarbyl substituted acylating agents described above such that these agents are not significantly involved in the reaction and the compositions of the invention do not contain significant amounts of additives derived from such agents. In some embodiments the components of the invention, or the compositions of the invention, may contain less than 10 percent by weight of these agents, or of the additives derived from these agents. In other embodiments the maximum allowable amount may be 5, 3, 2, 1 or even 0.5 or 0.1 percent by weight. One of the purposes of these embodiments is to allow the exclusion of agents such as polyisobutylene succinic anhydrides from the reactions of the invention and so, to also allow the exclusion of quaternized salt detergent additive derived from agents such as polyisobutylene succinic anhydrides. The focus of this invention is on polyester, or hyperdispersant, quaternary salt detergent additives.

The quaternizing agents useful in preparing the quaternized polyester salts described above include any of the quaternizing agents described above with regards to the other quaternized salts. In one embodiment, the quaternizing agent can be a hydrocarbyl epoxide in combination with an acid. Examples of hydrocarbyl epoxides include: ethylene oxide, propylene oxide, butylene oxide, styrene oxide and

## 15

combinations thereof. In one embodiment the quaternizing agent does not contain any styrene oxide.

In some embodiments the acid used with the hydrocarbyl epoxide may be a separate component, such as acetic acid. In other embodiments, for example when the hydrocarbyl acylating agent is a dicarboxylic acylating agent, no separate acid component is needed. In such embodiments, the detergent may be prepared by combining reactants which are essentially free of, or even free of, a separate acid component, such as acetic acid, and rely on the acid group of the hydrocarbyl acylating agent instead. In other embodiments, a small amount of an acid component may be present, but at <0.2 or even <0.1 moles of acid per mole of hydrocarbyl acylating agent.

In some embodiments the quaternizing agent of the invention does not contain any substituent group that contains more than 20 carbon atoms. In other words, in some embodiments the long substituent group that allows for the resulting additive to be organic soluble and thus useful for the purposes of this invention is not provided by the quaternizing agent but instead is brought to the additive by the non-quaternized detergents described above.

In certain embodiments the molar ratio of detergent having an amine functionality to quaternizing agent is 1:0.1 to 2, or 1:1 to 1.5, or 1:1 to 1.3.

In some embodiments the hydrocarbyl-substituted compound having a tertiary amino group used to prepare the quaternary salt includes: (1) the condensation product of a hydrocarbyl-substituted acylating agent and a compound having an oxygen or nitrogen atom capable of condensing with said acylating agent and said condensation product further having a tertiary amino group; (2) a polyalkene-substituted amine having at least one tertiary amino group; (3) a Mannich reaction product having a tertiary amino group, said Mannich reaction product being prepared from the reaction of a hydrocarbyl-substituted phenol, an aldehyde, and an amine; (4) a polyester containing a tertiary amino group; or any combination thereof.

In some embodiments the stabilizing component includes a poly(hydroxycarboxylic acid) amide salt derivative represented by the formula  $[Y-CO[O-A-CO]_n-Z_r-R^+]_m pX^{q-}$  wherein Y is hydrogen or a substituted or non-substituted hydrocarbyl group for example a hydroxy substituted hydrocarbyl group, A is a divalent hydrocarbyl group, n is from 1 to 100, m is from 1 to 4, q is from 1 to 4 and p is an integer such that pq=m, Z is a divalent bridging group which is attached to the carbonyl group through a nitrogen atom, r is 0 or 1, R+ is an ammonium group and Xq- is an anion. In some embodiments the A in the formula of the poly(hydroxycarboxylic acid) amide salt derivative is fully saturated.

In some embodiments these stabilizing components are represented by the formula  $[Y-[O-A-CO]_n-Z_r-R^+]_m pX^{q-}$  wherein Y is hydrogen, a hydrocarbyl group (e.g. H-A-CO-), a hydrocarbyl group optionally substituted (e.g. H-A- or HO-A-) for example a hydroxy substituted hydrocarbyl or hydrocarbyl group (e.g. HO-A-CO-), A is a divalent hydrocarbyl group, n is from 1 to 100, m is from 1 to 4, q is from 1 to 4 and p is an integer such that pq=m, Z is a divalent bridging group which is attached to the carbonyl group through a nitrogen atom, r is 0 or 1, R+ is an ammonium group and Xq- is an anion. In some embodiments the A in the formula of the poly(hydroxycarboxylic acid) amide salt derivative is fully saturated.

In still other embodiments these stabilizing components are represented by the formula  $[H-[O-A-CO]_{(n+1)}-Z_r-R^+]_m pX^{q-}$  wherein A is a divalent hydrocarbyl group, n is

## 16

from 1 to 100, m is from 1 to 4, q is from 1 to 4 and p is an integer such that pq=m, Z is a divalent bridging group which is attached to the carbonyl group through a nitrogen atom, r is 0 or 1, R+ is an ammonium group and Xq- is an anion. In some embodiments the A in the formula of the poly(hydroxycarboxylic acid) amide salt derivative is fully saturated.

The poly(hydroxycarboxylic acid) amide salt derivatives described above may also be referred to as hyperdispersants.

10 The R+ group in the formulas above may be a primary, secondary, tertiary or quaternary ammonium group. In some embodiments R+ is a quaternary ammonium group. In some embodiments R+ in the hyperdispersant formula above is represented by formula  $-N^+(R^2)(R^3)(R^4)$  wherein R<sup>2</sup>, R<sup>3</sup> and R<sup>4</sup> may be selected from hydrogen and alkyl groups such as methyl.

15 In the hyperdispersant formulas above A may be a divalent straight chain or branched hydrocarbyl group. A may be a substituted aromatic, aliphatic or cycloaliphatic straight chain or branched divalent hydrocarbyl group. In some embodiments A is an arylene, alkylene or alkenylene group, in particular an arylene, alkylene or alkenylene group containing in the range of from 4 to 25, 6 to 25, 8 to 24, 10 to 22, or even 12 to 20 carbon atoms. In some embodiments 20 there are at least 4, 6, or even 8 to 14 carbon atoms connected directly between the carbonyl group and the oxygen atom derived from the hydroxyl group. The optional substituents in the group A may be selected from hydroxy, halo or alkoxy groups, especially C<sub>1-4</sub> alkoxy groups.

25 In the hyperdispersant formulas above n is in the range of from 1 to 100 however the lower limit for n may also be 2 or 3. The upper limit for n may be 100, 60, 40 20 or even 10. In other words n may be selected from any of the following ranges: 1 to 100; 2 to 100; 3 to 100; 1 to 60; 2 to 60; 3 to 60; 1 to 40; 2 to 40; 3 to 40; 1 to 20; 2 to 20; 3 to 20; 1 to 10; 2 to 10; and 3 to 10.

30 In the hyperdispersant formulas above Y is an optionally substituted hydrocarbyl group. Y may be aryl, alkyl or alkenyl containing up to 50 carbon atoms, or in the range of from 7 to 25 carbon atoms. For example, the optionally substituted hydrocarbyl group Y may be conveniently selected from heptyl, octyl, undecyl, lauryl, heptadecyl, heptadecenyl, heptadecadienyl, stearyl, oleyl and linoleyl. Other examples of Y include C<sub>4-8</sub> cycloalkyls such as cyclohexyl; polycycloalkyls such as polycyclic terpenyl groups which are derived from naturally occurring acids such as abietic acid; aryls such as phenyl; aralkyls such as benzyl; and polaryls such as naphthyl, biphenyl, stilbenyl and phenylmethylphenyl. Y may contain one or more functional groups such as carbonyl, carboxyl, nitro, hydroxy, halo, alkoxy, amino, preferably tertiary amino (no N—H linkages), oxy, cyano, sulphonyl and sulphonyl. The majority of the atoms, other than hydrogen, in substituted hydrocarbyl groups are generally carbon, with the heteroatoms (e.g., oxygen, nitrogen and sulphur) generally representing only a minority, about 33% or less, of the total non-hydrogen atoms present. Those skilled in the art will appreciate that functional groups such as hydroxy, halo, alkoxy, nitro and cyano in a substituted hydrocarbyl group Y will displace one of the hydrogen atoms of the hydrocarbyl, whilst functional groups such as carbonyl, carboxyl, tertiary amino (—N—), oxy, sulphonyl and sulphonyl in a substituted hydrocarbyl group will displace a —CH— or —CH<sub>2</sub>— moiety of the hydrocarbyl. In some embodiments Y is unsubstituted or substituted by a group selected from hydroxy, halo or alkoxy group, for example a C<sub>1-4</sub> alkoxy group. In still further embodiments Y is a stearyl group, 12-hydroxystearyl group,

an oleyl group or a 12-hydroxyoleyl group, and that derived from naturally occurring oil such as tall oil fatty acid.

In the hyperdispersant formulas above Z may be an optionally substituted divalent bridging group represented by the formula: —N(R<sup>1</sup>)—B— wherein R<sup>1</sup> is hydrogen or a hydrocarbyl group and B is an optionally substituted alkylene group. Examples of hydrocarbyl groups that may represent R<sup>1</sup> include methyl, ethyl, n-propyl, n-butyl and octadecyl. Examples of optionally substituted alkylene groups that may represent B include ethylene, trimethylene, tetramethylene and hexamethylene. Examples of Z moieties include —NHCH<sub>2</sub>CH<sub>2</sub>—, —NHCH<sub>2</sub>C(CH<sub>3</sub>)<sub>2</sub>CH<sub>2</sub>— and —NH(CH<sub>2</sub>)<sub>3</sub>—.

In the hyperdispersant formulas above r is preferably 1, i.e. the poly(hydroxycarboxylic acid) amide salt derivative must contain the optionally substituted divalent bridging group Z.

The anion X<sup>q-</sup> in the hyperdispersant formulas above is not critical and can be any anion (or mixture of anions) suitable to balance the positive charge of the poly(hydroxycarboxylic acid) amide cation. The anion X<sup>q-</sup> may be a sulphur-containing anion, such as sulphate and sulphonate anions. However, in some embodiments the anion X<sup>q-</sup> is a non-sulphur-containing anion such as a non-sulphur-containing organic anion or inorganic anion. Non-limiting examples of suitable anions are OH<sup>-</sup>, CH<sup>-</sup>, NH<sub>3</sub><sup>-</sup>, HCO<sub>3</sub><sup>-</sup>, HCOO<sup>-</sup>, CH<sub>3</sub>COO<sup>-</sup>, H<sup>-</sup>, BO<sub>3</sub><sup>3-</sup>, CO<sub>3</sub><sup>2-</sup>, C<sub>2</sub>H<sub>3</sub>O<sub>2</sub><sup>-</sup>, HCO<sup>2-</sup>, C<sub>2</sub>O<sub>4</sub><sup>2-</sup>, HC<sub>2</sub>O<sub>4</sub><sup>-</sup>, NO<sub>2</sub><sup>-</sup>, NO<sub>3</sub><sup>-</sup>, N<sup>3-</sup>, NH<sub>2</sub><sup>-</sup>, O<sup>2-</sup>, O<sub>2</sub><sup>2-</sup>, BeF<sub>3</sub><sup>-</sup>, F<sup>-</sup>, Na<sup>+</sup>, [Al(H<sub>2</sub>O)<sub>2</sub>(OH)<sub>4</sub>]<sup>-</sup>, SiO<sub>3</sub><sup>-</sup>, SiF<sub>6</sub><sup>-</sup>, H<sub>2</sub>PO<sub>4</sub><sup>-</sup>, p<sup>3-</sup>, PO<sub>4</sub><sup>3-</sup>, HPO<sub>4</sub><sup>2-</sup>, Cl<sup>-</sup>, ClO<sub>3</sub><sup>-</sup>, ClO<sub>4</sub><sup>-</sup>, ClO<sup>-</sup>, KO<sup>-</sup>, SbOH<sub>6</sub><sup>-</sup>, SnCl<sub>6</sub><sup>2-</sup>, [SnTe<sub>4</sub>]<sup>4-</sup>, CrO<sub>4</sub><sup>2-</sup>, Cr<sub>2</sub>O<sub>7</sub><sup>2-</sup>, MnO<sub>4</sub><sup>-</sup>, NiCl<sub>6</sub><sup>2-</sup>, [Cu(CO<sub>3</sub>)<sub>2</sub>(OH)<sub>2</sub>]<sub>4-</sub>, AsO<sub>4</sub><sup>3-</sup>, Br<sup>-</sup>, BrO<sub>3</sub><sup>-</sup>, IO<sub>3</sub><sup>-</sup>, I<sup>-</sup>, CN<sup>-</sup>, OCN<sup>-</sup>, etc. Suitable anions may also include anions derived from compounds containing a carboxylic acid group (e.g. a carboxylate anion), anions derived from compounds containing a hydroxyl group (e.g. an alkoxide, phenoxide or enolate anion), nitrogen based anions such as nitrate and nitrite, phosphorus based anions such as phosphates and phosphonates, or mixtures thereof. Non-limiting examples of suitable anions derived from compounds containing a carboxylic acid group include acetate, oleate, salicylate anions, and mixtures thereof. Non-limiting examples of suitable anions derived from compounds containing a hydroxyl group include phenate anions, and mixtures thereof. In some embodiments the anion X<sup>q-</sup> is a non-sulfur-containing anion selected from the group consisting of OH, a phenate group, a salicylate group, an oleate group and an acetate group, and in still other embodiments the anion is OH.

The one or more poly(hydroxycarboxylic acid) amide salt derivatives may be obtained by reaction of an amine and a poly(hydroxycarboxylic acid) of formula Y—CO[O-A-CO]<sub>n</sub>—OH wherein Y is hydrogen or optionally substituted hydrocarbyl group, A is a divalent optionally substituted hydrocarbyl group and n is from 1 to 100, with an acid or a quaternizing agent. The Y, A and n in the poly(hydroxycarboxylic acid) formula may be defined as above for the poly(hydroxycarboxylic acid) amide salt derivative formula.

As used herein, the term "hydrocarbyl" represents a radical formed by removal of one or more hydrogen atoms from a carbon atom of a hydrocarbon (not necessarily the same carbon atoms in case more hydrogen atoms are removed). Hydrocarbyl groups may be aromatic, aliphatic, acyclic or cyclic groups. Preferably, hydrocarbyl groups are aryl, cycloalkyl, alkyl or alkenyl, in which case they may be straight-chain or branched-chain groups. Representative hydrocarbyl groups include phenyl, naphthyl, methyl, ethyl,

butyl, pentyl, methylpentyl, hexenyl, dimethylhexyl, octenyl, cyclooctenyl, methylcyclooctenyl, dimethylcyclooctyl, ethylhexyl, octyl, isoctyl, dodecyl, hexadecenyl, eicosyl, hexacosyl, triacontyl and phenylethyl. The phrase "optionally substituted hydrocarbyl" is used to describe hydrocarbyl groups optionally containing one or more "inert" heteroatom-containing functional groups. By "inert" is meant that the functional groups do not interfere to any substantial degree with the function of the compound.

10 In one embodiment at least one, or all of the poly(hydroxycarboxylic acid) amide salt derivatives are sulphur-containing derivatives. In such an embodiment, said derivatives may have a sulphur content of at most 2.5 wt. % for example from 0.1 to 2.0 wt. % or from 0.6 to 1.2 wt. % sulphur, as measured by ICP-AES, based on the total weight of said derivatives. In another embodiment of the present invention, the one or more poly(hydroxycarboxylic acid) amide salt derivatives are non-sulphur-containing derivatives.

15 20 The group (—O-A-CO—) in the poly(hydroxycarboxylic acid)s and amide salt derivatives thereof described above may be a 12-oxystearyl group, 12-oxyoleyl group or a 6-oxycaproyl group.

25 The amines which react with poly(hydroxycarboxylic acid)s to form poly(hydroxycarboxylic acid) amide intermediates may include those defined in WO 97/41092. The amine reactant may be a diamine, a triamine or a polyamine. Suitable examples include diamines selected from ethylenediamine, N,N-dimethyl-1,3-propanediamine, triamines and polyamines selected from diethylenetriamine, triethylenetetramine, tetraethylenepentamine, pentaethylenhexamine and tris(2-aminoethyl)amine.

30 35 40 The amidation between the amine reactant and the (poly(hydroxycarboxylic acid) may be carried out according to methods known to those skilled in the art, by heating the poly(hydroxycarboxylic acid) with the amine reactant, optionally in a suitable hydrocarbon solvent such as toluene or xylene, and azeotroping off the formed water. Said reaction may be carried out in the presence of a catalyst such as p-toluenesulphonic acid, zinc acetate, zirconium naphthenate or tetrabutyl titanate.

45 50 55 The poly(hydroxycarboxylic acid) amide intermediate formed from reaction of the amine and the poly(hydroxycarboxylic acid) is reacted with an acid or a quaternizing agent to form a salt derivative, according to well-known methods. Acids that may be used to form the salt derivative may be selected from organic or inorganic acids. Said acids are conveniently selected from carboxylic acids, nitrogen-containing organic and inorganic acids, sulphur-containing organic or inorganic acids (such as sulphuric acid, methanesulphonic acid and benzenesulphonic acid).

60 65 70 Quaternizing agents that may be used to form the salt derivative may be selected from dimethyl sulfate, a dialkyl sulphate having from 1 to 4 carbon atoms, an alkyl halide such as methyl chloride, methyl bromide, aryl halide such as benzyl chloride. In one embodiment the quaternizing agent is a sulphur-containing quaternizing agent, in particular dimethyl sulfate or a dialkyl sulphate having from 1 to 4 carbon atoms, for example dimethyl sulphate. Quaternization is a well-known method in the art. For example, quaternization using dimethyl sulphate is described in U.S. Pat. Nos. 3,996,059, 4,349,389 and GB 1 373 660.

75 80 85 In some embodiments the poly(hydroxycarboxylic acid) amide salt derivatives have a TBN (total base number) value of less than 10 or even less than 5 or less than 2 mg KOH per gram, as measured by ASTM D 4739. Examples of poly(hydroxycarboxylic acid) amide salt derivatives that are

available commercially include that available from Lubrizol under the trade designation "SOLSPERSE 17000" (a reaction product of poly(12-hydroxystearic acid) with N,N-dimethyl-1,3-propanediamine and dimethyl sulphate) and those available under the trade designations "CH-5" and "CH-7" from Shanghai Sanzheng Polymer Company.

In some embodiments the stabilizing component includes a high molecular weight polyetheramine, which may be prepared by reacting one unit of a hydroxy-containing hydrocarbyl compound with two or more units of butylene oxide to form a polyether intermediate, and aminating the polyether intermediate by reacting the polyether intermediate with an amine or with acrylonitrile and hydrogenating the reaction product of the polyether intermediate and acrylonitrile.

Suitable polyetheramines may contain two or more ether units and is generally prepared from a polyether intermediate. The polyether intermediate can be a reaction product of one unit of a hydroxy-containing hydrocarbyl compound with two or more units of butylene oxide. The hydroxy-containing hydrocarbyl compound can be an alcohol or an alkyl-substituted phenol where the alcohol or alkyl substituent of the phenol can have 1 to 50 carbon atoms, 6 to 30 carbon atoms in a second instance, and 8 to 24 carbon atoms in a third instance. The alcohol or alkyl substituent of the phenol can have a straight carbon chain, branched carbon chain, or a mixture thereof. The hydroxy-containing hydrocarbyl compound can contain one or more hydroxyl groups.

The polyether intermediate from the reaction of a hydroxy-containing hydrocarbyl compound and butylene oxide can have 2 to 100 repeating butylene oxide units, 5 to 50 repeating butylene oxide units in a second embodiment, and 15 to 30 repeating butylene oxide units in a third embodiment. U.S. Pat. No. 5,094,667 provides reaction conditions for preparing a polyether intermediate.

The high molecular weight polyetheramine of the present invention can be prepared from the above described polyether intermediate that is prepared from butylene oxide.

In one embodiment of the invention the polyetheramine is prepared by reacting the polyether intermediate derived from butylene oxide with acrylonitrile to form a nitrile that is then hydrogenated to form a 3-aminopropyl terminated polyether as described in U.S. Pat. No. 5,094,667.

In another embodiment of the invention the polyetheramine is prepared by reacting the polyether intermediate derived from butylene oxide with an amine in an amination reaction to give an aminated polyether as described in European Publication No. EP310875. The amine can be a primary or secondary monoamine, a polyamine containing an amino group with a reactive N—H bond, or ammonia.

The high molecular weight polyetheramine of the present invention can have a number average molecular weight of 300 or 350 to 5000, in another instance of 400 to 3500, and in further instances of 450 to 2500 and 1000 to 2000.

In another embodiment of the invention the high molecular weight polyetheramine of the present invention can be represented by the formula  $R(OCH_2CHR^1)_x A$  where R is a C<sub>6</sub> to C<sub>30</sub> alkyl group or a C<sub>6</sub> to C<sub>30</sub> alkyl-substituted phenyl group; R<sup>1</sup> is ethyl; x is a number from 5 to 50; and A is OCH<sub>2</sub>CH<sub>2</sub>CH<sub>2</sub>NH<sub>2</sub> or —NR<sup>2</sup>R<sup>3</sup> wherein R<sup>2</sup> and R<sup>3</sup> are independently hydrogen, a hydrocarbyl group, or  $-(R^4NR^5)_yR^6$  wherein R<sup>4</sup> is an alkylene group having 2 to 10 carbon atoms, R<sup>5</sup> and R<sup>6</sup> are independently hydrogen or a hydrocarbyl group, and y is a number from 1 to 7. Throughout this application an alkylene group is a divalent alkane group. In a further embodiment of the polyetheramine of the

invention, R is a C<sub>8</sub> to C<sub>24</sub> alkyl group, x is a number from 15 to 30, and A is —OCH<sub>2</sub>CH<sub>2</sub>CH<sub>2</sub>NH<sub>2</sub>.

In some embodiments the high molecular weight polyetheramine is represented by the formula  $R(OCH_2CHR^1)_x A$  wherein R is a C<sub>6</sub> to C<sub>30</sub> alkyl group or a C<sub>6</sub> to C<sub>30</sub> alkyl-substituted phenyl group; R<sup>1</sup> is ethyl; x is a number from 5 to 50; and A is —OCH<sub>2</sub>CH<sub>2</sub>CH<sub>2</sub>NH<sub>2</sub> or —NR<sup>2</sup>R<sup>3</sup> wherein R<sup>2</sup> and R<sup>3</sup> are independently hydrogen, a hydrocarbyl group, or  $-(R^4NR^5)_yR^6$  wherein R<sup>4</sup> is an alkylene group having 2 to 10 carbon atoms, R<sup>5</sup> and R<sup>6</sup> are independently hydrogen or a hydrocarbyl group, and y is a number from 1 to 7.

In some embodiments the stabilizing component includes an alkanolamine substituted phenol where the phenol contains a hydrocarbyl substituent. Suitable materials may be represented by the formula:



where R<sup>1</sup> is a hydrocarbyl group, R<sup>2</sup> is a hydrocarbylene group, each R<sup>3</sup> is independently a hydrocarbylene group, and each R<sup>4</sup> is independently a hydrogen or a hydrocarbylene group. In some embodiments R<sup>1</sup> contains from 1 to 20, 8 to 20, 8 to 16, 10 to 14 or even about 12 carbon atoms; R<sup>2</sup> contains from 1 to 8, 1 to 6, 1 to 4, at least 1 carbon atom, or even about 1 carbon atom; each R<sup>3</sup> group contains from 1 to 8, 1 to 6, 1 to 4, 2 to 4, at least 2 carbon atoms, or even about 2 carbon atoms and may be identical; and each R<sup>4</sup> group is hydrogen or a hydrocarbylene group that contains from 1 to 8, 1 to 6, 1 to 4, 2 to 4, at least 2 carbon atoms, or even about 2 carbon atoms and may be identical.

In some embodiments the stabilizing component includes a low molecular weight acylated nitrogen compound derived from an alkyl succinic anhydride and an alkanolamine.

The stabilizing component may be a low molecular weight acylated nitrogen compound, which in some embodiments may be described as an amino ester or an amino ester salt. These materials may be prepared from the reaction of an alkyl succinic anhydride and an alkanolamine combined at a ratio of 1:10 to 10:1, 1:5 to 5:1, 3:5 to 5:3, 1:2 to 2:1, 1:1. The alkyl group of the alkyl succinic anhydride can be a hydrocarbyl group containing from about 4 to about 18 carbon atoms; from about 6 to about 18 carbon atoms, from about 9 to about 18 carbon atoms and particularly from about 12 to about 18 carbon atoms. The alkyl group of the alkyl succinic anhydride can be saturated, unsaturated, branched, linear or mixtures thereof. In some embodiments the alkyl group is linear.

The alkyl succinic anhydride can be the reaction product of a branched or linear olefin having about 4 to about 18 carbon atoms; from about 6 to about 18 carbon atoms, from about 9 to about 18 carbon atoms and particularly from about 12 to about 18 carbon atoms and maleic anhydride. This reaction is well known to those skilled in the art. Suitable examples of the alkyl succinic anhydride include dodecenyl succinic anhydride, pentadecenyl succinic anhydride, hexadecenyl succinic anhydride, octadecenyl succinic anhydride, heptadecenyl succinic anhydride, and the like.

The alkanolamine component of the acylated nitrogen compound of the present invention can be an amino alcohol, such as, an ethanolamine (including mono, di and tri ethanolamines), or a propanol amines (including mono, di and tri ethanolamines) in which nitrogen is attached directly to the carbon of the alkyl alcohol. Examples of the alkanolamine component of the acylated nitrogen compounds can include: monoethanolamine, triethanolamine, methylethanolamine, methyldiethanolamine, dimethylethanolamine, diethylethanolamine, dibutylethanolamine, monoisopropanolamine, diisopropanolamine, triisopropanolamine. The examples of these alkanolamines are well known to those skilled in the art. In some embodiments the alkanolamine used in the preparation of the compatibilizer is triethanolamine, N,N-dimethylaminopropanol, N,N-diethylaminopropanol, N,N-dimethylethanol amine, N,N-diethylaminobutanol, N,N,N-tris(hydroxyethyl)amine, or a mixture thereof.

The reaction products of the alkyl succinic anhydride or its acid or ester derivative and the alkanolamine include amides, imides, esters, amine salts, ester-amides, ester-amine salts, amide-amine salts, acid-amides, acid-esters and mixtures thereof. The reaction and the resulting products of the alkyl succinic anhydride and the alkanolamine are readily known to those skilled in the art.

The stabilizing component may be an aromatic carboxylic acid/amine salt or an abietic acid/amine salt. That is a salt of an aromatic carboxylic acid and/or an abietic acid with a fatty amine. However in other embodiments, these moderately performing stabilizing compounds may be excluded from the compositions of the invention, or at least required in higher amounts than some of the other stabilizing compounds described in order to provide comparable performance. This is some embodiments these materials are part of the invention and in other embodiments these materials may be treated more as comparative examples, at least where more consistent performance is required and/or at lower concentration levels.

The aromatic carboxylic acid may include an aliphatic moiety containing the carboxylic acid group, and the aliphatic moiety may contain from 1 to 26 or more carbon atoms, or from 1 to 10 carbon atoms. Alternatively, the aromatic carboxylic acid may be one in which the carboxylic group is bonded directly to the aromatic moiety, for example benzoic acid. Suitable aromatic carboxylic acids include benzoic acid, phenylacetic acid, phenylpropionic acid, phenylbutyric acid, phenylpentanoic acid, phenylhexanoic acid, phenylheptanoic acid, phenyloctanoic acid, phenylnonanoic acid, phenyldecanoic acid, phenyldodecanoic acid, phenyltetradecanoic acid, phenylhexadecanoic acid, and phenyloctadecanoic acid.

The aromatic carboxylic acid may also include phenyl versions of any of the acids described above, where a hydroxy group is present on the aromatic ring, generally adjacent to the aliphatic moiety containing the carboxylic acid group. Examples of acids include salicylic acid.

The acid moiety of the amine salt may contain a hydroxy group, an oxy group, or it may contain an ester moiety. Hydroxy carboxylic acids include phenyl hydroxy carboxylic acids having a hydroxy alkyl group which may contain from 3 to 26 carbon atoms. The phenyl or other aryl ring or rings may include one or more substituents attached thereto including alkyl groups of 1 to 12 or 10 more carbon atoms, alkoxy groups containing from 1 to 12 carbon atoms, hydroxy, carbamyl, carboalkyloxy, amido or amino alkyl groups.

When one substituent group is present, not counting the hydroxy group of a phenyl ring as a substituent if present, it

may generally be in a position para to the carboxylic acid moiety. When two or more substituents are present, they may generally be in a position 3,4 or 3,5 on a phenyl ring. Illustrative examples include meta or para toluic acid, meta- or para-hydroxybenzoic acid, anisic acid and gallic acid.

The amine suitable for use in the preparation of the salt are not overly limited and may include any alkyl amine, though generally are fatty acid amines derived from fatty carboxylic acids. The alkyl group present in the amine may contain from 10 to 30 carbon atoms, or from 12 to 18 carbon atoms, and may be linear or branched. In some embodiments the alkyl group is linear and unsaturated. Typical amines include pentadecylamine, octadecylamine, cetylamine, oleylamine, decylamine, dodecylamine, dimethyldodecylamine, tridecylamine, heptadecylamine, octadecylamine, stearylamine, and any combination thereof. In some embodiments the fatty amine salt is a salt of a salicylic acid and oleylamine. In some embodiments the fatty amine may be described as a fatty acid derived amine salt, for example a salt of a salicylic acid and oleylamine.

The salt is re prepared in any suitable manner and generally includes mixing the amines and acid under conditions designed to avoid conversion to the amide, ester, or other condensation products. In one embodiment, substantially equal molar proportions of the mine and acid are used. However, when desired, an excess of the amine may be employed, in which case the proportions may be in the range of from about 1.0 to about 1.2 mole proportions of amine per mole proportion of acid.

In some embodiments the stabilizing component is a fatty acid amino salicylate, that is an amine salt of salicylic acid where the amine used in the preparation of the salt is derived from a fatty acid.

Amines suitable for use in the preparation of the amino salicylate are not overly limited and may include any alkyl amine, though generally are fatty acid amines derived from fatty carboxylic acids. The alkyl group present in the amine may contain from 10 to 30 carbon atoms, or from 12 to 18 carbon atoms, and may be linear or branched. In some embodiments the alkyl group is linear and unsaturated. Typical amines include pentadecylamine, octadecylamine, cetylamine, oleylamine, decylamine, dodecylamine, dimethyldodecylamine, tridecylamine, heptadecylamine, octadecylamine, stearylamine, and any combination thereof. In some embodiments the fatty acid derived amine salt of a salicylic acid of oleylamine.

Any of the stabilizing components described above may be used alone, even to the exclusion of one or more the components listed, while in other embodiments they may be used in any combination of two or more thereof.

Useful compatibilizers may be described more generally as a compound having at least one hydrogen-donating group, a least one hydrogen-accepting group, and at least one hydrocarbyl group, where the hydrogen-donating group and the hydrogen-accepting group are not separated by more than 8 bonds, where the bond counted may include covalent bonds or ionic bonds, and generally both types of bonds combined.

In some embodiments the hydrocarbyl group of the compatibilizer compound is sufficient to impart solubility to the compatibilizer in the medium in which it is used, while in other embodiments it contains at least 8, 10, 14 or even 20 carbon atoms. In still other embodiments the hydrocarbyl group of the compatibilizer compound may be any of the hydrocarbyl groups defined above related to the compatibilizer component.

A hydrogen-donating group is a substituent group or atom capable of donating a proton to another compound. The group may itself be described as a hydrogen donor group. Suitable examples of hydrogen-donating groups which are included in the invention are: —OH, —OR, —C(O)OH, —C(O)OR, —SH, —NRH, —NH<sub>2</sub>, —NR<sub>2</sub>H, —NRH<sub>2</sub>, and —NH<sub>3</sub>, where each R is independently a hydrocarbyl group. Suitable examples may have a positive charge.

A hydrogen-accepting group is a substituent group or atom capable of accepting a proton. The group may itself be described as a hydrogen acceptor group. Suitable examples of hydrogen-accepting groups which are included in the invention are: =O, —C(O)OH, —C(O)OR, =S, —NRH, —NRR, —NHH where each R is independently a hydrocarbyl group; a carboxylic acid derivative such as a carboxylate anion, an imide, an amide, an imidazoline, an anhydride or an ester; or a phosphate or thiophosphate. Additional examples of hydrogen-accepting groups include the anions described above. Suitable examples may have a negative charge.

In other embodiments the accepting and donating groups discussed above are separated by at least 1 to no more than 6, 7 or 8 bonds, at least 2 or even 3 to no more than 6, 7 or 8, and even no less than 2 up to no more than 4 bonds. In some embodiments the compatibilizer compound contains at least one set of groups, that is at least one acceptor group and at least one donating group, but in other embodiments the compatibilizer compounds may contain multiple sets of groups. For example the compatibilizer compounds may include at least two acceptor groups and at least two donating groups, or even more. Useful compatibilizer compounds may include 1 set of accepting and donating groups, two sets, or even three sets of groups. While not wishing to be bound by theory it is believed that the greater the number of sets of accepting and donating groups, the better a compounds performance as a compatibilizer, however the distance between the groups, as measured by the number of bonds between the groups also has an impact on compatibilizer performance. In addition it is believed that the functionality of the accepting and donating groups can be impaired if they are sterically hindered.

Suitable compatibilizers may contain: (i) a single hydrogen-acceptor group and a single hydrogen-donating groups; (ii) a single hydrogen-acceptor group and two or more hydrogen-donating groups; (iii) two or more hydrogen-acceptor groups and one hydrogen-donating group; or (iv) two or more hydrogen-acceptor groups and two or more hydrogen-donating groups.

In some embodiments the compatibilizer component includes (i) a compound having at least one set of accepting and donating groups separated by less than 4 bonds, where bonds include both covalent and ionic bonds, (ii) a compound having at least one hydrogen-acceptor group such as a nitrogen atom and at least two, or even three hydrogen-donating groups, such as —OH groups, separated by 1 to 8 bonds, (iii) a compound having at least two sets of accepting and donating groups where the groups of each set are separated by 1 to 8 bonds, where bonds include both covalent and ionic bonds, or any combination thereof.

The stabilizing component of the invention may essentially free of or even free of any of the following types of materials: (i) an overbased detergent with a metal to substrate ratio of greater than 3:1, including borated versions thereof; (ii) an alkyl imidazoline; (iii) a hydrocarbyl phosphoric acid or acid ester, a hydrocarbyl thiophosphoric acid or acid ester, a hydrocarbyl dithiophosphoric acid or acid ester, an amine salt of one or more of these acids and acids

esters, or combinations thereof; (iv) an alkylbenzene sulfonate or derivatives thereof; or combinations thereof.

In some embodiments component (c), the stabilizing component, is essentially free or even free of compounds represented by the formula:



or salted versions thereof wherein: X¹ is O or NR⁵ where R¹ and R⁵ can optionally link to form a ring; R³ is H or a hydrocarbyl; R⁴ is H, a hydrocarbyl group, —CH<sub>2</sub>C(O)—X² where X² is —OH, or where R⁴ is linked with R² to form a ring where the linked —R⁴—R²— group is —CH<sub>2</sub>C(O)—; and wherein each R¹ is independently H, a hydrocarbyl group or —(CH<sub>2</sub>CH<sub>2</sub>NH)<sub>n</sub>—H where n is an integer from 1 to 10; where each R² is independently H, a hydrocarbyl group or —(CH<sub>2</sub>CH<sub>2</sub>NH)<sub>n</sub>—H where n is 1 to 10, or where R² is linked with R⁴ to form a ring where the linked —R⁴—R²—group is —CH<sub>2</sub>C(O)—; and R⁵ is a hydrocarbyl group; with the proviso that at least one of R¹, R², R³, R⁴, or R⁵ is a hydrocarbyl group and wherein the entire compound contains at least 10 carbon atoms. In some embodiments at least one of R¹, R², R³, R⁴, or R⁵ is a hydrocarbyl group that contains at least 10 carbon atoms.

In still further embodiments component (c), the stabilizing component, is free of compounds represented by one or more of the following formulas:



wherein each R⁶ is independently a hydrocarbyl group; each X³ is independently a nitrogen containing group derived from a polyethylene polyamine; and n may be an integer from 1 to 10.

In some embodiments the stabilizing component excludes certain nitrogen-containing dispersants or borated version thereof. For example the computerize component of the invention may be essentially free or even free of nitrogen-containing dispersants, or borated versions thereof, which are the reaction product of a hydrocarbyl-substituted succinic acylating agent and a polyamine but which do not contain a quaternized nitrogen atom.

In one embodiment, component (c), the stabilizing component, is free of borated non-quaternized succinimide dispersants derived from the reaction of boric acid, a mixture of polyethylene polyamines and/or bottoms, and a polyisobutylene succinic anhydride derived from conventional PIB; borated succinimide non-quaternized dispersants derived from the reaction of boric acid, a mixture of polyethylene polyamines and/or bottoms, and polyisobutylene

succinic anhydrides derived from high vinylidene PIB; borated non-quaternized dispersants derived from the reaction of a polyisobutylene succinimide dispersant and boric acid where the dispersant is derived from a mixture of polyethylene polyamines and/or bottoms, and a polyisobutylene succinic anhydride derived from conventional PIB; a non-borated non-quaternized polyisobutylene succinimide dispersant derived from a polyisobutylene succinic anhydride derived from high vinylidene PIB and TEPA; a non-borated alkyl imidazoline derived from a polyalkylene amine and a fatty mono-carboxylic acid.

In some embodiments the stabilizing component of the invention is free of overbased detergents. In some embodiments the stabilizing component of the invention is free of alkyl imidazolines. In some embodiments the stabilizing component of the invention is free of phosphorus containing additives, such as hydrocarbyl phosphates, hydrocarbyl thio-phosphates, and dihydrocarbyl dithiophosphates.

In some embodiments the stabilizing component of the present invention is essentially free to free of compounds represented by the formula:



wherein: X<sup>1</sup> is an oxygen atom, a sulfur atom a hydrocarbylene group or —NR<sup>2</sup>; X<sup>2</sup> is an oxygen atom or a sulfur atom; X<sup>3</sup> is ═P(OR<sup>2</sup>)<, or ═S(O)<; and Y is —R<sup>2</sup>, or —OR<sup>2</sup>; each R<sup>1</sup> is a hydrocarbylene group; each R<sup>2</sup> is independently a hydrocarbyl group or —H; and each n is independently 0 or 1. In some embodiments the stabilizing component of the present invention includes a salted version of one or more of the compound described above. In any of the embodiments described above, X<sup>2</sup> of the formula above may also be a hydrocarbyl group and X<sup>3</sup> may be ═C< where the hydrocarbyl group of X<sup>2</sup> may be attached to the carbon atom of X<sup>3</sup> by either a double bond as shown in the formula or but a single bond. In still other embodiments, X<sup>2</sup> of the formula above is a hydrocarbyl group and X<sup>3</sup> is ═C< while the n for the [R<sup>1</sup>] group is 0. Various stabilizing components, including many of those described above, fall under this formula and/or at least one of its described embodiments.

#### INDUSTRIAL APPLICATION

The present invention includes a process of preparing a composition that includes combining: (a) a medium comprising a solvent, a functional fluid, or combinations thereof; (b) a friction modifier component that includes a compound containing one or more amide functional groups that is not fully soluble in the medium; and (c) a stabilizing component that is soluble in (a) and that interacts with (b) such that (b)'s solubility in (a) is improved where the stabilizing component includes a compound having at least one hydrogen-donating group, a least one hydrogen-accepting group, and at least one hydrocarbyl group, where the hydrogen-donating group and the hydrogen-accepting group are not separated by more than 8 covalent and ionic bonds. The processes of the present invention involve adding components (b) and (c) to component (a) and mixing the components so that particles of components (b) and (c) have an average diameter of less than 10 microns. The processes of the present invention results in a mixture that is clear and/or stable in that the friction modifier does not drop out of

solution, does not make the mixture appear cloudy or hazy, stays suspended, dispersed and/or dissolved in the mixture, or combinations thereof, or that at least shows improvement in one or more of these areas when compared to an identical composition that does not contain the stabilizing component.

While not wishing to be bound by theory, it is believed that in at least some embodiments the compositions of the present invention improve the stability and/or compatibility of the friction modifier component in the overall composition due to the friction modifier component being solubilized in a complex with the compatibilizer.

In some embodiments the processes of the present invention result in a mixture with an improved clarity, as defined by a lower JTU and/or NTU value, compared to the same composition that does not contain the stabilizing component.

As noted above, components (b) and (c) may be present in component (a) in the form of dispersed particles having an average diameter of less than 10 microns. In some embodiments the particles have an average diameter of less than 10, 5 or 3 microns. In other embodiments, the particles have an average diameter of from 0.01, 0.02, 0.03 or 0.09 to 10, 6, 5 or 3 microns. In some embodiments 80% of the particles meet one or more of the size limitations described above. In other embodiments 90%, 95%, 99% or even 100% of the particles meet the size limits. The means by which the particles are formed is not overly limited, and may include the mixing of components (a), (b) and (c) using conventional equipment and/or techniques.

In some embodiments the compositions of the present invention and/or the compositions that result from the processes of the present invention include both finished functional fluids and additive concentrates. Finished functional fluids are fluids that are ready for use. Additive concentrates are compositions that may contain all of the additives required for a finished fluid, but in concentrated form. This makes shipment and handling easier. At the appropriate time, the additive concentrate may be blended with a fluid, solvent, or similar diluent, as well as additional additives, to produce a finished functional fluid that is ready for use.

When referring to finished functional fluids, the compositions involved with the present invention may include: from 1, 3 or 10 to 99, 80 or 70 percent by weight of component (a), the medium; from 0.1, 0.2, 0.3, 0.5 or 1.0 to 10, 7.5, 5, 4 or 3 percent by weight of component (b), the friction modifier; and from 0.1, 0.2, 0.3, 0.5 or 2.0 to 20, 10, 8, 5, 4 or 2 percent by weight of component (c), the stabilizing component.

When referring to additive concentrates, the compositions involved with the present invention may include: from 0.1, 1, 3 or 10 to 90, 60, 50, 30, or 20 percent by weight of component (a), the medium; from 0.1, 0.5, 1, 5 or 8 to 60, 30, 20 or 10 percent by weight of component (b), the friction modifier; and from 0.1, 0.2, 0.3, 0.5 or 2.0 to 20, 10, 8, 5, 4 or 2 percent by weight of component (c), the stabilizing component. As noted above in some embodiments the medium and the stabilizing component may be the same material, in which case the dual functioning material may be present in any of the ranges provided above for either component (a) or (c).

In some embodiments the compositions of the present invention are formed by mixing components (b) and (c) into component (a) such that component (b) forms small particles within component (a) and component (c) acts to stabilize these particles. In some embodiments component (c) and component (b) form mixed particles in component (a). In some embodiments some or all of the particles formed are

within the sizes described above. In other embodiments, some or even all of the particles are larger than those described above.

In some embodiments the components of the present invention are mixed by conventional means. The amount of mixing required varies from composition to composition and is that sufficient to produce the particles of the desired size and/or stability. In some embodiments the mixing may be accomplished by milling the components and in still other embodiments the mixing may be accomplished by milling the components at low temperature.

The mixing may be in the form of a milling process using conventional milling equipment and techniques. However, in some embodiments the milling is completed at low temperatures, in some embodiments from at less than 30 degrees C. and in other embodiments from -10, 0 or 5 to 30, 25 or 20 degrees C. The low temperature milling may be achieved by cooled milling equipment, pre-cooled components, adding a chilling agent such as dry ice (solid carbon dioxide) to the components during milling, or a combination thereof. The resulting compositions in some embodiments may be described as stable dispersions and in other embodiments may be described as solubilized solutions, or even combinations thereof, where the main difference between such embodiments may be the size of the particles involved.

In other embodiments the compositions of present invention are not formed by milling or any other high-energy input methods, but rather are formed with simple mixing and very little mechanical energy input.

In some embodiments the functional fluid with which the compositions of the invention are used is a fuel. The fuel compositions of the present invention comprise the stabilized compositions described above and a liquid fuel, and is useful in fueling an internal combustion engine or an open flame burner. These compositions may also contain one or more additional additives described herein. In some embodiments, the fuels suitable for use in the present invention include any commercially available fuel, and in some embodiments any commercially available diesel fuel and/or biofuel.

The description that follows of the types of fuels suitable for use in the present invention refer to the fuel that may be present in the additive containing compositions of the present invention as well as the fuel and/or fuel additive concentrate compositions to which the additive containing compositions may be added.

Fuels suitable for use in the present invention are not overly limited. Generally, suitable fuels are normally liquid at ambient conditions e.g., room temperature (20 to 30° C.) or are normally liquid at operating conditions. The fuel can be a hydrocarbon fuel, non-hydrocarbon fuel, or mixture thereof.

The hydrocarbon fuel can be a petroleum distillate, including a gasoline as defined by ASTM specification D4814, or a diesel fuel, as defined by ASTM specification D975. In one embodiment the liquid fuel is a gasoline, and in another embodiment the liquid fuel is a non-leaded gasoline. In another embodiment the liquid fuel is a diesel fuel. The hydrocarbon fuel can be a hydrocarbon prepared by a gas to liquid process to include for example hydrocarbons prepared by a process such as the Fischer-Tropsch process. In some embodiments, the fuel used in the present invention is a diesel fuel, a biodiesel fuel, or combinations thereof.

Suitable fuels also include heavier fuel oils, such as number 5 and number 6 fuel oils, which are also referred to as residual fuel oils, heavy fuel oils, and/or furnace fuel oils.

Such fuels may be used alone or mixed with other, typically lighter, fuels to form mixtures with lower viscosities. Bunker fuels are also included, which are generally used in marine engines. These types of fuels have high viscosities and may be solids at ambient conditions, but are liquid when heated and supplied to the engine or burner it is fueling.

The non-hydrocarbon fuel can be an oxygen containing composition, often referred to as an oxygenate, which includes alcohols, ethers, ketones, esters of a carboxylic acids, nitroalkanes, or mixtures thereof. Non-hydrocarbon fuels can include methanol, ethanol, methyl t-butyl ether, methyl ethyl ketone, transesterified oils and/or fats from plants and animals such as rapeseed methyl ester and soybean methyl ester, and nitromethane.

Mixtures of hydrocarbon and non-hydrocarbon fuels can include, for example, gasoline and methanol and/or ethanol, diesel fuel and ethanol, and diesel fuel and a transesterified plant oil such as rapeseed methyl ester and other bio-derived fuels. In one embodiment the liquid fuel is an emulsion of water in a hydrocarbon fuel, a non-hydrocarbon fuel, or a mixture thereof.

In several embodiments of this invention the liquid fuel can have a sulphur content on a weight basis that is 50,000 ppm or less, 5000 ppm or less, 1000 ppm or less, 350 ppm or less, 100 ppm or less, 50 ppm or less, or 15 ppm or less.

The liquid fuel of the invention is present in a fuel composition in a major amount that is generally greater than 95% by weight, and in other embodiments is present at greater than 97% by weight, greater than 99.5% by weight, greater than 99.9% by weight, or greater than 99.99% by weight.

The compositions described above may also include one or more additional additives. Such additives include oxidation inhibitors and antioxidants, friction modifiers antiwear agents, corrosion inhibitors, or viscosity modifiers, as well as dispersant and detergents different from those described above. These additional additives may be present in the medium, particularly when the medium includes a functional fluid. When present, these additional additives may represent from 0, 0.1, 0.5 or 1 to 2, 5, 10 or 15 percent of the overall composition, when considering a finished fluid, and from 0, 0.5, 1 or 2 to 4, 10, 20 or 40 percent of the overall composition, when considering an additive concentrate.

As allowed for by the ranges above, in one embodiment, the additive concentrate may comprise the additives of the present invention and be substantially free of any additional solvent. In these embodiments the additive concentrate containing the additives of the present invention is neat, in that it does not contain any additional solvent added to improve the material handling characteristics of the concentrate, such as its viscosity.

As used herein, the terms hydrocarbyl and/or hydrocarbylene substituent and/or group are used in their ordinary sense, which is well-known to those skilled in the art. Specifically, each refers to a group having a carbon atom directly attached to the remainder of the molecule and having predominantly hydrocarbon character. Examples include: hydrocarbon substituents, that is, aliphatic (e.g., alkyl or alkenyl), alicyclic (e.g., cycloalkyl, cycloalkenyl) substituents, and aromatic-, aliphatic-, and alicyclic-substituted aromatic substituents, as well as cyclic substituents wherein the ring is completed through another portion of the molecule (e.g., two substituents together form a ring); substituted hydrocarbon substituents, that is, substituents containing non-hydrocarbon groups which, in the context of this invention, do not alter the predominantly hydrocarbon nature of the substituent (e.g., halo (especially chloro and

fluoro), hydroxy, alkoxy, mercapto, alkylmercapto, nitro, nitroso, and sulfoxy); hetero substituents, that is, substituents which, while having a predominantly hydrocarbon character, in the context of this invention, contain other than carbon in a ring or chain otherwise composed of carbon atoms. Heteroatoms include sulfur, oxygen, nitrogen, and encompass substituents as pyridyl, furyl, thieryl and imidazolyl. In general, no more than two, preferably no more than one, non-hydrocarbon substituent will be present for every ten carbon atoms in the hydrocarbyl group; typically, there will be no non-hydrocarbon substituents in the hydrocarbyl group. The term hydrocarbyl and/or hydrocarbylene may also have the definition provided in the sections above.

It is known that some of the materials described above may interact in the final formulation, so that the components of the final formulation may be different from those that are initially added. For instance, metal ions (of, e.g., a detergent) can migrate to other acidic or anionic sites of other molecules. In addition the acylating agents and/or substituted hydrocarbon additives of the present invention may form salts or other complexes and/or derivatives, when interacting with other components of the compositions in which they are used. The products formed thereby, including the products formed upon employing the composition of the present invention in its intended use, may not be susceptible of easy description. Nevertheless, all such modifications and reaction products are included within the scope of the present invention; the present invention encompasses the composition prepared by admixing the components described above.

As allowed for by the ranges above, in one embodiment, the additive concentrate may comprise the additives of the present invention and be substantially free of any additional solvent. In these embodiments the additive concentrate containing the additives of the present invention is neat, in that it does not contain any additional solvent added to improve the material handling characteristics of the concentrate, such as its viscosity.

Unless otherwise indicated all percent values and ppm values herein are weight percent values and/or calculated on a weight basis.

## EXAMPLES

The invention will be further illustrated by the following examples, which sets forth particularly advantageous embodiments. While the examples are provided to illustrate the present invention, they are not intended to limit it

### Example Set A

A set of samples is prepared by adding a specific friction modifier to specific mediums where the friction modifier is known to have compatibility issues in such compositions. The friction modifier used in this testing is an alkylene amide friction modifier derived from oleic acid (FM-1). The mediums used in this testing include: a heavy aromatic petroleum distillate solvent (MEDIUM-1) and a commercially available gasoline (MEDIUM-2). The compatibilizers used in this testing include: a mineral oil control that does not contain any sets of hydrogen-donating and accepting groups (COMPAT-1), an alkyl amine alkyl phenol where the alkyl group attached to the phenol is derived from 1000 number average molecular weight polyisobutylene and the alkyl amine group attached to the phenol is derived from a dialkylamine where the compound has a single hydrogen-accepting group separated by at least 4 bonds from a single hydrogen-donating group (COMPAT-2), a quaternary

ammonium salt derived from a 1000 number average molecular weight polyisobutylene derived succinic anhydride and a polyalkylene polyamine, quaternized using an alkylene epoxide in combination with an acid where the compounds has a hydrogen-donating group within two bonds of two hydrogen-accepting groups and a second hydrogen-donating group separated by one bond from a hydrogen-accepting group (COMPAT-3), a low molecular weight acylated nitrogen compound that includes a hydrogen-accepting group within three bonds of two hydrogen-donating groups (COMPAT-4), and two alkyl polyoxyalkyl amine compound that includes a hydrogen-accepting group within 3 bonds of a hydrogen donating group having different molecular weights: a higher molecular weight compound (COMPAT-5), and a lower molecular weight compound (COMPAT-6).

Each example is heated up to 80 degrees Celsius and stirred and then held at temperature for 1 hour. Each sample is then cooled to 23 degrees C. and stored, with the clarity of each sample being checked at set time intervals. Each example is visually evaluated to check for cloudiness, haziness and even for drop out of the friction modifier.

The results from the example set are provided in the tables below:

TABLE 1

| Formulations <sup>1</sup> and Results <sup>2</sup> in Neat Compositions |                |               |               |               |               |               |
|-------------------------------------------------------------------------|----------------|---------------|---------------|---------------|---------------|---------------|
|                                                                         | Comp<br>Ex 1-1 | Inv<br>Ex 1-2 | Inv<br>Ex 1-3 | Inv<br>Ex 1-4 | Inv<br>Ex 1-5 | Inv<br>Ex 1-6 |
| MEDIUM-1                                                                |                |               |               |               |               |               |
| MEDIUM-2                                                                |                |               |               |               |               |               |
| FM-1                                                                    | 30             | 30            | 30            | 30            | 30            | 30            |
| COMPAT-1                                                                | 70             |               |               |               |               |               |
| COMPAT-2                                                                |                | 70            |               |               |               |               |
| COMPAT-3                                                                |                |               | 70            |               |               |               |
| COMPAT-4                                                                |                |               |               | 70            |               |               |
| COMPAT-5                                                                |                |               |               |               | 70            |               |
| COMPAT-6                                                                |                |               |               |               |               | 70            |
| 1 DAY                                                                   | SOLID          | SOLID         | SOLID         | SOLID         | SOLID         | SOLID         |
| 1 WEEK                                                                  | SOLID          | SOLID         | SOLID         | SOLID         | SOLID         | SOLID         |

<sup>1</sup>All formulation values in Table 1 are percent by weight. The compatibilizers tested may contain an inherent amount of diluent such as a diluent oil.

<sup>2</sup>Empty cells in the results section indicate no rating was taken for that sample at that time. A "Clear" rating indicates the sample gelled. A "SOLID" rating indicates more than half of the sample does not flow within 30 seconds of being inverted.

TABLE 2

| Formulations <sup>1</sup> and Results <sup>2</sup> in Solvent Compositions |                   |               |               |               |               |               |
|----------------------------------------------------------------------------|-------------------|---------------|---------------|---------------|---------------|---------------|
|                                                                            | Comp<br>Ex 2-1    | Inv<br>Ex 2-2 | Inv<br>Ex 2-3 | Inv<br>Ex 2-4 | Inv<br>Ex 2-5 | Inv<br>Ex 2-6 |
| MEDIUM-1                                                                   | 85                | 50            | 50            | 50            | 50            | 50            |
| MEDIUM-2                                                                   |                   |               |               |               |               |               |
| FM-1                                                                       | 15                | 15            | 15            | 15            | 15            | 15            |
| COMPAT-1                                                                   |                   |               |               |               |               |               |
| COMPAT-2                                                                   |                   | 35            |               |               |               |               |
| COMPAT-3                                                                   |                   |               | 35            |               |               |               |
| COMPAT-4                                                                   |                   |               |               | 35            |               |               |
| COMPAT-5                                                                   |                   |               |               |               | 35            |               |
| COMPAT-6                                                                   |                   |               |               |               |               | 35            |
| 1 DAY                                                                      | Heavy<br>Sediment | SOLID         | Suspension    | Hazy          | SOLID         | SOLID         |

<sup>1</sup>All formulation values in Table 1 are percent by weight. The compatibilizers tested may contain an inherent amount of diluent such as a diluent oil.

<sup>2</sup>Empty cells in the results section indicate no rating was taken for that sample at that time. A "Clear" rating indicates the sample was clear with no sediment, suspension or solid dropout. A "Heavy Sediment" rating indicates a large amount of sediment dropped out of the sample. A "Suspension" rating indicates large particles are visible throughout the sample. A "Hazy" rating indicates light is able to pass through the sample but it is not clear. A "SOLID" rating indicates more than half of the sample does not flow within 30 seconds of being inverted.

TABLE 3

| Formulations <sup>1</sup> and Results <sup>2</sup> in Gasoline Compositions |                    |               |               |               |               |               |
|-----------------------------------------------------------------------------|--------------------|---------------|---------------|---------------|---------------|---------------|
|                                                                             | Comp<br>Ex 3-1     | Inv<br>Ex 3-2 | Inv<br>Ex 3-3 | Inv<br>Ex 3-4 | Inv<br>Ex 3-5 | Inv<br>Ex 3-6 |
| MEDIUM-1                                                                    |                    |               |               |               |               |               |
| MEDIUM-2                                                                    | 99.95              | 99.66         | 99.66         | 99.66         | 99.66         | 99.66         |
| FM-1                                                                        | 0.05               | 0.05          | 0.05          | 0.05          | 0.05          | 0.05          |
| COMPAT-1                                                                    |                    |               |               |               |               |               |
| COMPAT-2                                                                    |                    | 0.12          |               |               |               |               |
| COMPAT-3                                                                    |                    |               | 0.12          |               |               |               |
| COMPAT-4                                                                    |                    |               |               | 0.12          |               |               |
| COMPAT-5                                                                    |                    |               |               |               | 0.12          |               |
| COMPAT-6                                                                    |                    |               |               |               |               | 0.12          |
| 1 DAY                                                                       | Fine<br>Suspension | Clear         | Clear         | Clear         | Clear         | Clear         |
| 1 WEEK                                                                      |                    | Clear         | Clear         | Clear         | Clear         | Clear         |
| 2 WEEKS                                                                     |                    | Clear         | Clear         | Clear         | Clear         | Clear         |
| 3 WEEKS                                                                     |                    | Clear         | Clear         | Clear         | Clear         | Clear         |
| 4 WEEKS                                                                     |                    | Clear         | Clear         | Clear         | Clear         | Clear         |

<sup>1</sup>All formulation values in Table 1 are percent by weight. The compatibilizers tested may contain an inherent amount of diluent such as a diluent oil.

<sup>2</sup>Empty cells in the results section indicate no rating was taken for that sample at that time. A "Clear" rating indicates the sample was clear with no sediment, suspension or solid dropout. A "Fine Suspension" rating indicates fine particles are visible throughout the sample.

The results show that the inventive compatibilizers of the invention improve the compatibility of FM-1 in neat additive concentrates (where the medium of each example is the diluent inherently present in the compatibilizer itself), in solvent diluted compositions, and in gasoline compositions where the lack of compatibility of the friction modifier is evident in the comparative example even at very low concentrations.

#### Example Set B

A set of samples is prepared according to the procedures described in Example SET A above. The friction modifier used in this testing is an alkylene amide friction modifier derived from stearic acid (FM-2). The mediums used in this testing are MEDIUM-1 as described above and MEDIUM-2 as described above. The compatibilizers used in this testing include: COMPAT-1 as described above, COMPAT-2 as described above, COMPAT-3 as described above, COMPAT-4 as described above, COMPAT-5 as described above, and COMPAT-6 as described above.

Each example is prepared and evaluated using the procedures described above in Example set A.

The results from the example set are provided in the tables below:

TABLE 4

| Formulations <sup>1</sup> and Results <sup>2</sup> in Neat Compositions |                |               |               |               |               |               |
|-------------------------------------------------------------------------|----------------|---------------|---------------|---------------|---------------|---------------|
|                                                                         | Comp<br>Ex 4-1 | Inv<br>Ex 4-2 | Inv<br>Ex 4-3 | Inv<br>Ex 4-4 | Inv<br>Ex 4-5 | Inv<br>Ex 4-6 |
| MEDIUM-1                                                                |                |               |               |               |               |               |
| MEDIUM-2                                                                |                |               |               |               |               |               |
| FM-2                                                                    | 30             | 30            | 30            | 30            | 30            | 30            |
| COMPAT-1                                                                | 70             |               |               |               |               |               |
| COMPAT-2                                                                |                | 70            |               |               |               |               |
| COMPAT-3                                                                |                |               | 70            |               |               |               |
| COMPAT-4                                                                |                |               |               | 70            |               |               |
| COMPAT-5                                                                |                |               |               |               | 70            |               |
| COMPAT-6                                                                |                |               |               |               |               | 70            |
| 1 DAY                                                                   | SOLID          | SOLID         | SOLID         | SOLID         | SOLID         | SOLID         |
| 1 WEEK                                                                  | SOLID          | SOLID         | SOLID         | SOLID         | SOLID         | SOLID         |
| 2 WEEK                                                                  | SOLID          | SOLID         | SOLID         | SOLID         | SOLID         | SOLID         |

TABLE 4-continued

| Formulations <sup>1</sup> and Results <sup>2</sup> in Neat Compositions |                |               |               |               |               |               |
|-------------------------------------------------------------------------|----------------|---------------|---------------|---------------|---------------|---------------|
|                                                                         | Comp<br>Ex 4-1 | Inv<br>Ex 4-2 | Inv<br>Ex 4-3 | Inv<br>Ex 4-4 | Inv<br>Ex 4-5 | Inv<br>Ex 4-6 |
| 5                                                                       |                |               |               |               |               |               |
| 3 WEEK                                                                  | SOLID          | SOLID         | SOLID         | SOLID         | SOLID         | SOLID         |
| 4 WEEK                                                                  | SOLID          | SOLID         | SOLID         | SOLID         | SOLID         | SOLID         |

<sup>1</sup>All formulation values in Table 1 are percent by weight. The compatibilizers tested may contain an inherent amount of diluent such as a diluent oil.

<sup>2</sup>Empty cells in the results section indicate no rating was taken for that sample at that time. A "Clear" rating indicates the sample was clear with no sediment, suspension or solid dropout. A "SOLID" rating indicates more than have of the sample does not flow within 30 seconds of being inverted.

TABLE 5

| Formulations <sup>1</sup> and Results <sup>2</sup> in Solvent Compositions |                |               |               |               |               |               |
|----------------------------------------------------------------------------|----------------|---------------|---------------|---------------|---------------|---------------|
|                                                                            | Comp<br>Ex 5-1 | Inv<br>Ex 5-2 | Inv<br>Ex 5-3 | Inv<br>Ex 5-4 | Inv<br>Ex 5-5 | Inv<br>Ex 5-6 |
| 20                                                                         | MEDIUM-1       | 85            | 50            | 50            | 50            | 50            |
| MEDIUM-2                                                                   |                |               |               |               |               |               |
| FM-2                                                                       | 15             | 15            | 15            | 15            | 15            | 15            |
| COMPAT-1                                                                   |                |               |               |               |               |               |
| COMPAT-2                                                                   |                |               | 35            |               |               |               |
| COMPAT-3                                                                   |                |               |               | 35            |               |               |
| COMPAT-4                                                                   |                |               |               |               | 35            |               |
| COMPAT-5                                                                   |                |               |               |               |               | 35            |
| COMPAT-6                                                                   |                |               |               |               |               |               |
| 1 DAY                                                                      | SOLID          | SOLID         | SOLID         | SOLID         | SOLID         | SOLID         |

<sup>1</sup>All formulation values in Table 1 are percent by weight. The compatibilizers tested may contain an inherent amount of diluent such as a diluent oil.

<sup>2</sup>Empty cells in the results section indicate no rating was taken for that sample at that time. A "Clear" rating indicates the sample was clear with no sediment, suspension or solid dropout. A "Heavy Sediment" rating indicates a large amount of sediment dropped out of the sample. A "Suspension" rating indicates large particles are visible throughout the sample. A "Hazy" rating indicates light is able to pass through the sample but it is not clear. A "SOLID" rating indicates more than have of the sample does not flow within 30 seconds of being inverted.

TABLE 6

| Formulations <sup>1</sup> and Results <sup>2</sup> in Solvent Compositions |                   |               |               |                   |                   |                   |
|----------------------------------------------------------------------------|-------------------|---------------|---------------|-------------------|-------------------|-------------------|
|                                                                            | Comp<br>Ex 6-1    | Inv<br>Ex 6-2 | Inv<br>Ex 6-3 | Inv<br>Ex 6-4     | Inv<br>Ex 6-5     | Inv<br>Ex 6-6     |
| 40                                                                         | MEDIUM-1          | 92.5          | 75            | 75                | 75                | 75                |
| MEDIUM-2                                                                   |                   |               |               |                   |                   |                   |
| FM-2                                                                       | 7.5               | 7.5           | 7.5           | 7.5               | 7.5               | 7.5               |
| COMPAT-1                                                                   |                   |               |               |                   |                   |                   |
| COMPAT-2                                                                   |                   |               | 17.5          |                   |                   |                   |
| COMPAT-3                                                                   |                   |               |               | 17.5              |                   |                   |
| COMPAT-4                                                                   |                   |               |               |                   | 17.5              |                   |
| COMPAT-5                                                                   |                   |               |               |                   |                   | 17.5              |
| COMPAT-6                                                                   |                   |               |               |                   |                   |                   |
| 1 DAY                                                                      | Heavy<br>Sediment | Clear         | Clear         | Heavy<br>Sediment | Heavy<br>Sediment | Heavy<br>Sediment |

<sup>1</sup>All formulation values in Table 1 are percent by weight. The compatibilizers tested may contain an inherent amount of diluent such as a diluent oil.

<sup>2</sup>Empty cells in the results section indicate no rating was taken for that sample at that time. A "Clear" rating indicates the sample was clear with no sediment, suspension or solid dropout. A "Heavy Sediment" rating indicates a large amount of sediment dropped out of the sample. A "Suspension" rating indicates large particles are visible throughout the sample. A "Hazy" rating indicates light is able to pass through the sample but it is not clear. A "SOLID" rating indicates more than have of the sample does not flow within 30 seconds of being inverted.

The results show that the inventive compatibilizers of the invention improve the compatibility of FM-1 in solvent diluted compositions compared to examples that contain no compatibilizer as well as examples that contain non-inventive compatibilizers.

Each of the documents referred to above is incorporated herein by reference. Except in the Examples, or where otherwise explicitly indicated, all numerical quantities in this description specifying amounts of materials, reaction

conditions, molecular weights, number of carbon atoms, and the like, are to be understood as modified by the word "about."

Unless otherwise indicated, each chemical or composition referred to herein should be interpreted as being a commercial grade material which may contain the isomers, by-products, derivatives, and other such materials which are normally understood to be present in the commercial grade. However, the amount of each chemical component is presented exclusive of any solvent or diluent, which may be customarily present in the commercial material, unless otherwise indicated. It is to be understood that the upper and lower amount, range, and ratio limits set forth herein may be independently combined. Similarly, the ranges and amounts for each element of the invention can be used together with ranges or amounts for any of the other elements. As used herein, the expression "consisting essentially of" permits the inclusion of substances that do not materially affect the basic and novel characteristics of the composition under consideration.

We claim:

1. A composition comprising:

- (a) a medium comprising a solvent, a functional fluid, an additive concentrate or combinations thereof; and
- (b) greater than 0.2 percent to about 10 percent by weight of a friction modifier component comprising oleamide or stearylamide; and
- (c) about 0.5 to about 20 percent by weight of a stabilizing component that is soluble in (a) and that interacts with (b) such that (b)'s solubility in (a) is improved, said stabilizing component comprising:

(i) a quaternary ammonium salt comprising the reaction product of (a) an 800-1600 Mn polyisobutylene-substituted succinic anhydride with a polvalkylenepolyamine, quaternized using (b) a hydrocarbyl epoxide in combination with an acid or mixtures thereof, or

(iii) a poly(hydroxycarboxylic acid) amide salt derivative represented by the formula  $[Y-CO(O-A-CO)]_n-Z_r-R^+)_m pX^{q-}$  wherein Y is hydrogen, a hydrocarbyl group or a substituted hydrocarbyl group, A is a divalent hydrocarbyl group, n is from 1 to 100, m is from 1 to 4, q is from 1 to 4 and p is an integer such that pq=m, Z is a divalent bridging group which is attached to the carbonyl group through a nitrogen atom, r is 0 or 1, R<sup>+</sup> is an ammonium group and X<sup>q-</sup> is an anion, wherein the poly(hydroxycarboxylic acid) is a condensation product of 12-hydroxystearic acid, ricinoleic acid, 12-hydroxy dodecanoic acid, 5-hydroxy dodecanoic acid, 5-hydroxy decanoic acid, 4-hydroxy decanoic acid, 10-hydroxy undecanoic acid, or combinations thereof; or

(vi) a low molecular weight acylated nitrogen compound derived from an alkyl succinic anhydride and an alkanolamine comprising N,N-dimethylamino-propanol, N,N-diethylaminopropanol, N,N-dimethyl ethanolamine, or N,N-diethylaminobutanol, wherein the alkyl group contains from about 4 to about 18 carbon atoms;

wherein components (b) and (c), or (b) alone, are present in component (a) in the form of dispersed particles having an average diameter of less than 10 microns; and

wherein the stabilizing component comprises a compound having at least one hydrogen-donating group, a least one hydrogen-accepting group, and at least one hydro-

carbyl group, where the hydrogen-donating group and the hydrogen-accepting group are not separated by more than 8 bonds, wherein said bonds include covalent and ionic bonds.

5 2. The composition of claim 1 wherein the hydrocarbyl-substituted compound having a tertiary amino group used to prepare the quaternary salt comprises:

- (1) the condensation product of a hydrocarbyl-substituted acylating agent and a compound having an oxygen or nitrogen atom capable of condensing with said acylating agent and said condensation product further having a tertiary amino group;
- (2) a polyalkene-substituted amine having at least one tertiary amino group;
- (3) a Mannich reaction product having a tertiary amino group, said Mannich reaction product being prepared from the reaction of a hydrocarbyl-substituted phenol, an aldehyde, and an amine;
- (4) a polyester containing a tertiary amino group; or any combination thereof.

15 3. The composition of claim 1 wherein the turbidity of the overall composition is improved, as defined by a lower JTU and/or NTU value compared to the same composition that does not contain (c), the stabilizing component.

20 4. The composition of claim 1 wherein (b), the friction modifier component, comprises a compound represented by the formula:



30 wherein: X<sup>4</sup> is an oxygen atom or a sulfur atom; and each R<sup>2</sup> and R<sup>3</sup> is independently a hydrogen or a hydrocarbyl group.

35 5. The composition of claim 1 wherein the friction modifier further comprises a compound derived from a hydroxycarboxylic acid.

40 6. The composition of claim 1 wherein the friction modifier further comprises oleyl tartrimide, stearyl tartrimide, 2-ethylhexyl tartrate, or combinations thereof.

45 7. The composition of claim 1 wherein the amount of component (b) in the overall composition is at least 0.5 percent by weight.

50 8. A process of preparing a clear and stable composition comprising:

- (a) a medium comprising a solvent, a functional fluid, an additive concentrate, or combinations thereof; and
- (b) greater than 0.2 percent to about 10 percent by weight of a friction modifier component comprising oleamide or stearylamide; and
- (c) about 0.5 to about 20 percent by weight of a stabilizing component that is soluble in (a) and that interacts with (b) such that (b)'s solubility in (a) is improved; said method comprising the steps of:

- I. adding components (b) and (c) to component (a);
- II. mixing the components so that components (b) are present in component (a) in the form of dispersed particles having an average diameter of less than 10 microns; and

55 wherein the stabilizing component comprises a compound having at least one hydrogen-donating group, a least one hydrogen-accepting group, and at least one hydrocarbyl group, where the hydrogen-donating group and the hydrogen-accepting group are not separated by more

than 8 bonds, wherein said bonds include covalent and ionic bonds, said stabilizing component comprising:

- (i) a quaternary ammonium salt comprising the reaction product of (a) an 800-1600 Mn polyisobutylene-substituted succinic anhydride with a polyalkylene polyamine, quaternized using (b) a hydrocarbyl epoxide in combination with an acid or mixtures thereof, or
- (iii) a poly(hydroxycarboxylic acid) amide salt derivative represented by the formula  $[Y-CO[O-A-CO]_n-Z_r-R^+]_m pX^{q-}$  wherein Y is hydrogen, a hydrocarbyl group or a substituted hydrocarbyl group, A is a divalent hydrocarbyl group, n is from 1 to 100, m is from 1 to 4, q is from 1 to 4 and p is an integer such that pq=m, Z is a divalent bridging group which is attached to the carbonyl group through a nitrogen atom, r is 0 or 1, R<sup>+</sup> is an ammonium group and X<sup>q-</sup> is an anion, wherein the poly(hydroxycarboxylic acid) is a condensation product of 12-hydroxystearic acid, ricinoleic acid, 12-hydroxydodecanoic acid, 5-hydroxydodecanoic acid, 5-hydroxydecanoic acid, 4-hydroxydecanoic acid, 10-hydroxyundecanoic acid, or combinations thereof; or
- (vi) a low molecular weight acylated nitrogen compound derived from an alkyl succinic anhydride and an alkanolamine comprising N,N-dimethylamino-propanol, N,N-diethylaminopropanol, N,N-dimethyl ethanolamine, or N,N-di ethylaminobutanol, wherein the alkyl group contains from about 4 to about 18 carbon atoms.

9. The process of claim 8 wherein the clarity of the resulting mixture is improved, as defined by a lower JTU and/or NTU value compared to the same composition that does not contain (c), the stabilizing component. 35

10. The process of claim 8 wherein (b), the friction modifier component, comprises a compound represented by the formula: 35



wherein: X<sup>4</sup> is an oxygen atom or a sulfur atom; and each R<sup>2</sup> and R<sup>3</sup> is independently a hydrogen or a hydrocarbyl group.

10 11. The composition of claim 1 wherein (b), the friction modifier, comprises C<sub>8</sub>-C<sub>24</sub> aliphatic monocarboxylic amide.

12. The composition of claim 1 wherein (b), the friction modifier, comprises oleyl amide or stearyl amide or combinations thereof.

15 13. The composition of claim 1 wherein (c), the stabilizing component, comprises a quaternary ammonium salt derived from a polyisobutylene-derived succinic anhydride and a polyalkenene polyamine, quaternized using an alkylene epoxide in combination with an acid.

20 14. The composition of claim 1 wherein (b) the friction modifier, is present in an amount of about 0.1 to about 10 percent by weight.

25 15. The composition of claim 1 wherein (b), the friction modifier, comprises a C<sub>8</sub>-C<sub>24</sub> aliphatic monocarboxylic amide and is present in an amount of greater than 0.2 to about 10 percent by weight.

16. A composition comprising:

(a) a medium comprising a solvent, a functional fluid, an additive concentrate or combinations thereof; and

(b) about 0.3 to about 0.5 percent by weight of oleamide, and

(c) about 1.3 to about 2.0 percent by weight of a stabilizing component comprising a reaction product of poly(12-hydroxystearic acid) with N,N-dimethyl-1,3-propanediamine and dimethyl sulphate;

wherein components (b) and (c), or (b) alone, are present in component (a) in the form of dispersed particles having an average diameter of less than 10 microns.

\* \* \* \* \*